



US005827606A

# United States Patent [19]

Marumoto et al.

[11] Patent Number: 5,827,606

[45] Date of Patent: Oct. 27, 1998

[54] **LOW ELECTRIC NOISE ELECTRODE SYSTEM**[75] Inventors: **Ikuro Marumoto**, Anjyo; **Taisuke Miyamoto**, Okazaki; **Satoru Tojo**, Toshio Asahi, both of Toyota; **Hiroshi Morita**, Toyota; **Iwao Hibino**, Toyota; **Kimitoshi Murata**, Toyota; **Nobuyuki Ishihara**, Toyota, all of Japan[73] Assignee: **Toyota Jidosha Kabushiki Kaisha**, Toyota, Japan

[21] Appl. No.: 610,975

[22] Filed: Mar. 1, 1996

## Related U.S. Application Data

[63] Continuation of Ser. No. 278,970, Jul. 22, 1994, abandoned.

## Foreign Application Priority Data

|               |      |       |          |
|---------------|------|-------|----------|
| Jul. 22, 1993 | [JP] | Japan | 5-202662 |
| Nov. 19, 1993 | [JP] | Japan | 5-290835 |
| Mar. 1, 1994  | [JP] | Japan | 6-031262 |
| Jul. 5, 1994  | [JP] | Japan | 6-153857 |

[51] **Int. Cl.<sup>6</sup>** ..... B32B 3/00; B32B 9/00[52] **U.S. Cl.** ..... 428/209; 428/210; 428/688; 428/701; 428/702; 428/901[58] **Field of Search** ..... 428/209, 901, 428/210, 688, 701, 702

## References Cited

### U.S. PATENT DOCUMENTS

3,992,230 11/1976 Komiyama et al. .

|           |         |                   |
|-----------|---------|-------------------|
| 4,091,245 | 5/1978  | Komiyama et al. . |
| 4,217,470 | 8/1980  | Kirner .          |
| 4,419,547 | 12/1983 | Imai et al. .     |
| 5,102,720 | 4/1992  | Raj ..... 428/209 |

## FOREIGN PATENT DOCUMENTS

|           |         |           |
|-----------|---------|-----------|
| 27 58 502 | 11/1978 | Germany . |
| 40 15 487 | 11/1990 | Germany . |
| 42 23 684 | 1/1993  | Germany . |
| 54-38446  | 3/1979  | Japan .   |
| 54-50735  | 4/1979  | Japan .   |
| 58-23278  | 2/1983  | Japan .   |
| 59-23074  | 2/1984  | Japan .   |
| 61-53461  | 3/1986  | Japan .   |
| 1-22472   | 4/1989  | Japan .   |

Primary Examiner—Patrick Ryan

Assistant Examiner—Cathy F. Lam

Attorney, Agent, or Firm—Oblon, Spivak, McClelland, Maier &amp; Neustadt, P.C.

## ABSTRACT

In the electrode for preventing noise electric wave according to the present invention in which the resistivity of the second layer is larger than that of the first layer, it is possible to prevent the generation of noise electric wave. In the electrode for preventing noise electric wave according to the present invention in which the layer for preventing noise electric wave has the porosity of not more than 20%, it is possible to prevent the radio noise. In the electrode for preventing noise electric wave according to the present invention in which the high-fusing conductive material layer exists between the substrate and the resisting material layer, it is possible to prevent the formation of the concave portion.

20 Claims, 22 Drawing Sheets



FIG. 1



FIG. 2



FIG. 3



FIG. 4



FIG. 5



FIG. 6



FIG. 7



FIG. 9





FIG. 8

FIG. 10



FIG. 11



LEVEL OF NOISE ELECTRIC WAVE (dB $\mu$ V/m)

(180 MHz)

PERFORMANCE AT  
INITIAL STAGEPERFORMANCE AT  
24 HOURS LATER

FIG. 12

FIG. 13



FIG. 14



FIG. 15



FIG. 16



FIG. 17



FIG. 18



FIG. 19



FIG. 20



FIG. 21



FIG. 22



FIG. 23



FIG. 24



FIG. 25



FIG. 26



FIG. 27



FIG. 28



FIG. 29



FIG. 30



FIG. 31



FIG. 32



FIG. 33



FIG. 34



FIG. 35



LEVEL OF NOISE ELECTRIC WAVE (dB $\mu$ V/m)

FIG. 36



FIG. 37

LEVEL OF NOISE ELECTRIC WAVE (dB $\mu$ V/m)

(800-HOUR DURABLE PRODUCT : 180MHz)

THICKNESS OF HIGH-FUSING CONDUCTIVE MATERIAL LAYER ( $\mu$ m)LEVEL OF NOISE ELECTRIC WAVE (dB $\mu$ V/m)

(800-HOUR DURABLE PRODUCT : 180MHz)

THICKNESS OF HIGH-FUSING CONDUCTIVE MATERIAL LAYER ( $\mu$ m)

FIG. 38



28... COVERING PORTION

LEVEL OF NOISE ELECTRIC WAVE (dB $\mu$ V/m)

FIG. 39

LEVEL OF NOISE  
ELECTRIC WAVE (dB $\mu$ V/m)

FIG. 40



LEVEL OF NOISE ELECTRIC WAVE (dB $\mu$ V/m)

FIG. 41

EFFICIENCY AT INITIAL STAGE



FIG. 42



FIG. 43



FIG. 44



FIG. 45



FIG. 46



## LOW ELECTRIC NOISE ELECTRODE SYSTEM

This application is a Continuation of application Ser. No. 08/278,970, filed on Jul. 22, 1994, now abandoned.

### BACKGROUND OF THE INVENTION

#### 1. Field of the Invention

This invention relates to an electrode for preventing noise electric wave and a method thereof which prevents the generation of noise electric wave, especially, the generation of noise electric wave for the radio which is loaded on automobiles and the like. The electrode according to the present invention is used as a rotor electrode of distributor of automobiles.

#### 2. Description of the Related Art

In conventional distributor of an internal combustion of automobiles, a rotor electrode rotates to intermittently oppose a side-fixed electrode having a small clearance between them. The rotor electrode and the side-fixed electrode discharge between them so that they feed a number of ignition plugs. However, in this conventional feeding method, noise electric wave (ignition noise) is generated due to spark discharge between the rotor electrode and the side-fixed electrode. Since the noise electric wave has wide and high frequency band, it causes hindrance on radiocommunication such as TV or radio, electronic equipments loaded on automobiles and the like; for example, EFI (electronical controlled fuel injection apparatus), ESC (electronic skid control apparatus), EAT (electronic control automatic transmission).

As shown in FIG. 45, the above spark discharge current comprises capacity discharge current and induction discharge current. The capacity discharge current is high-frequency current which flows for 10 micron seconds from the beginning of discharge at the initial discharge stage due to rapid build-up. The induction discharge current is low-frequency current (about 10 to 100 mA) which continuously flows for 500 to 1500 micron seconds soon after the capacity discharge current flows.

Ignition energy supplied for the ignition plug is proportionated with the product of the induction discharge current and its discharge duration. Concerning the induction discharge current, since the absolute value level of the current value is low, it has little influence on the noise electric wave. Therefore, in order to effectively prevent the noise electric wave without decreasing the ignition energy, it is important that the starting voltage and the capacity discharge current are firmly decreased.

Conventionally, various measures for preventing noise electric wave have been taken. For example, a method for placing the resistor outside or inside of the plug, a method for introducing resistance to a part of high-voltage wiring, a method for establishing a condenser in order to prevent noise. However, in these methods, effects are not sufficient and reliability is deteriorated.

Japanese Patent Registration No. 858984 discloses that high electrical resistance substance is formed on the surface of the discharge electrode in order to prevent the generation of noise electric wave caused by discharge gap. However, in this method, only 5 to 6 dB of noise can be decreased so that required performance cannot be achieved.

Japanese Unexamined Patent Publication No. 50735/1979 discloses the technique in which the discharge electrode which is one element of ignition distributor of internal

combustion is performed by surface treatment so that the starting voltage and the capacity discharge current are decreased, thereby preventing noise electric wave. In this technique, mixed powder comprising CuO (cupric oxide) and  $Al_2O_3$  (alumina) is thermal sprayed on the surface of the discharge electrode to form the layer for preventing noise electric wave. Thus, the layer for prevention of noise electric wave is formed on the surface of the discharge electrode which is faced to an opposite electrode. In the electrode for preventing noise electric wave, preliminary micro discharge is generated between CuO as oxide resistor and  $Al_2O_3$  as oxide dielectric substance, so main discharge voltage generated between CuO and the opposite electrode is reduced, thereby decreasing the capacity discharge current. The effect of the preliminary micro discharge is called as Malter effect, and the method for preventing noise electric wave which makes use of Malter effect is recently noticed.

Japanese Examined Patent Publication No. 22472/1989 discloses one example of the electrode for preventing noise electric wave which makes use of Malter effect. This electrode comprises an electrode substrate and a resistive material layer coated on the surface of the electrode substrate which is faced to the opposite electrode. The resistive material layer is made of semi-conductive alumina-ceramics material. The resistive material layer is formed on the surface of the electrode substrate because titania ( $TiO_2$ ) is added to oxide ceramics mainly comprising alumina ( $Al_2O_3$ ), and reducing treatment is performed in reducing atmosphere. In the electrode for preventing noise electric wave, preliminary micro discharge is generated between titania having semi-conductivity (resistivity) and alumina as dielectric substance, so main discharge voltage generated between the electrode for preventing noise electric wave and the opposite electrode is reduced, thereby decreasing the capacity discharge current.

However, in the method for preventing noise electric wave which makes use of Malter effect, the effect for preventing noise electric wave is not sufficient so that more effect is required. As a result, a bonding wire or a H/T code for prevention of noise electric wave is required. Therefore, there are disadvantages in cost and assembling manhour.

When the conventional electrode for preventing noise electric wave disclosed in Japanese Unexamined Patent Publication No. 50735/1979 is applied for a rotor electrode of distributor, noise is generated in the radio loaded on automobiles. In this case, radio noise is terrible as compared with the case in which the rotor electrode without layer (thermal sprayed layer) for preventing noise electric wave is used.

Since the radio is easily influenced by electric wave and electric noise, the radio loaded on automobiles has PNL (Pulse Noise Limiter) function in order to control noise generation due to ignition noise. The PNL function is the function in which ignition noise in sound signal is absorbed by shutting the gate for a predetermined time (about 20 micron seconds) when the pulse noise above the predetermined level is input through antenna.

There are two kinds of rotor electrodes: one is the rotor electrode in which the layer (thermal sprayed layer) for preventing noise electric wave is formed on the surface of the rotor electrode faced to the opposite electrode by use of the normal thermal spraying method that thermal spraying is performed in the direction perpendicular to the surface, and the other is the rotor electrode without the layer. FIG. 46 shows the difference of electric wave form between them at the time of induction discharge.  $Al_2O_3+60$  wt % CuO is used as thermal spraying material.

As shown in FIG. 46, as compared with the rotor electrode without the layer, in the rotor electrode with the layer (thermal sprayed layer) for preventing noise electric wave, induction discharge in which the absolute level of the current value is high can be maintained for a long time. In accordance with this, PNL operating time becomes longer. There are interrelation between the PNL operating time and the level of the radio noise. Therefore, in the electrode with the layer for preventing noise electric wave which is formed by use of the normal thermal spraying method, the radio noise becomes deteriorated.

Inventors have studied the cause of deterioration of the radio noise in the rotor electrode with the layer (thermal sprayed layer) for preventing noise electric wave, and they have found that the porous part in the thermal sprayed layer have bad influence on the radio noise.

When the thermal sprayed layer has the porous part, much amount of micro discharge is generated between thermal spraying materials at the time of discharge, and relatively large induction discharge current continuously flows for a long time. As a result, the pulse noise caused by induction discharge current is input into the radio, and the PNL function repeats ON/OFF action of the gate for a long time. Therefore, the pulse noise input from the antenna of the radio is cut off, but the radio noise due to the repeated ON/OFF action of the gate in PNL circuit is generated. For example, when induction discharge current continuously flows for 1000 micro seconds, the PNL function repeats ON/OFF action of the gate about 50 times to firmly generate the radio noise.

The porous part in the thermal sprayed layer results from the method for thermal spraying. Namely, in the process for thermal spraying on the surface of the rotor electrode faced to the opposite electrode, thermal spraying is performed in the direction perpendicular to the surface. At this time, the thermal spraying materials are adhered to the surface which is perpendicular to the thermal spraying direction, and also to the surface which is horizontal to the thermal spraying direction. Therefore, thick thermal spraying layer is formed on the surface which is perpendicular to the thermal spraying direction, and the porous thermal spraying layer is formed on the surface which is horizontal to the thermal spraying direction.

In the conventional electrode for preventing noise electric wave disclosed in Japanese Examined Patent Publication No. 22472/1989, there are drawbacks in the durability. When the conventional electrode had been used for a long time, electric noise (radiation field intensity) had been increased, and required efficiency level could not be obtained.

In order to study the cause of the above problems, inventors have observed the discharge generating situation. As a result, although the resistive material layer having high electric resistive value has a close distance from the opposite electrode, discharge is not generated at the resistive material layer. Only at the part of the electrode substrate having low electric resistive value which is near the opposite electrode, namely, at the portion of the electrode substrate which is near a boundary portion between the electrode substrate and the resistive material layer, discharge is generated. Inventors have examined the relationship between the discharge generating situation and noise electric generating situation, and they found that the discharge generating situation is closely related to the durability of the electrode for preventing noise electric wave. When discharge is generated at the portion of the electrode substrate which is near the boundary portion

between the electrode substrate and the resistive material layer, the electrode substrate is fused by heat at the time of discharge since the electrode substrate comprises metal materials having lower fusing point than that of ceramics. 5 Inventors have found that the temperature at the time of discharge reaches about 1300° to 1500° C. sectionally. As a result, when the electrode had been used for a long time, a concave portion is formed at the portion of the electrode substrate which is near the boundary portion between the electrode substrate and the resistive material layer due to fused loss, and discharge is generated at the bottom of the concave portion. Then, discharge is hard to occur, or micro discharge is frequently occurred and relatively large induction discharge current continuously flows since the discharge passage becomes complicated. Therefore, noise electric 10 15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9920 9925 9930 9935 9940 9945 9950 9955 9960 9965 9970 9975 9980 9985 9990 9995 10000 10005 10010 10015 10020 10025 10030 10035 10040 10045 10050 10055 10060 10065 10070 10075 10080 10085 10090 10095 10100 10105 10110 10115 10120 10125 10130 10135 10140 10145 10150 10155 10160 10165 10170 10175 10180 10185 10190 10195 10200 10205 10210 10215 10220 10225 10230 10235 10240 10245 10250 10255 10260 10265 10270 10275 10280 10285 10290 10295 10300 10305 10310 10315 10320 10325 10330 10335 10340 10345 10350 10355 10360 10

substrate; a first layer comprising oxide dielectric substance and oxide resistor, and being formed on the surface of the substrate faced to an opposite electrode; and a second layer comprising oxide dielectric substance and oxide resistor, being formed on the surface of the first layer faced to the opposite electrode, and having larger resistivity than that of the first layer.

In the above electrodes for preventing noise electric wave, the method for forming the first layer and the second layer is not restricted, and various methods for forming the layer can be applied, for example, plasma spraying method, ion plating method, sputtering method and so on. However, when the second layer comprising metal oxide and having larger resistivity than that of the first layer is formed on the surface of the first layer comprising metal oxide, considering the cost, it is preferable that the second layer is formed on the surface of the first layer by performing oxidation treatment on the surface of the first layer.

The method for producing the electrode for preventing noise electric wave comprises a process for forming a first layer which comprises metal oxide on the surface of a substrate faced to an opposite electrode, and a process for forming a second layer which comprises metal oxide and has larger resistivity than that of the first layer on the surface of the first layer faced to the opposite electrode by performing oxidation treatment on the surface of the first layer.

The electrode for preventing noise electric wave and for solving the above first and second objects comprises an electrode substrate; and a layer for preventing noise electric wave comprising thermal sprayed layer, being coated on the surface of the electrode substrate faced to an opposite electrode, and having the porosity of not more than 20%.

Materials of the layer for preventing noise electric wave are not especially restricted, and high electric resistive material or electric insulating material can be used alone or in combinations. Furthermore, semi-conductive material can be used. Concretely, the high electric resistive materials include CuO, Cr<sub>2</sub>O<sub>3</sub>, NiO, ZnO and so on; the electric insulating materials include Al<sub>2</sub>O<sub>3</sub>, SiO<sub>2</sub>, ZrO<sub>2</sub>, MgO and so on; the semiconductive materials include FeO, Fe<sub>2</sub>O<sub>3</sub>, TiO<sub>2</sub>, ferrite and so on. It is preferable that oxides are used as materials of the layer for preventing noise electric wave in order to prevent oxidation deterioration due to discharge in the atmosphere.

The electrode for preventing noise electric wave can be manufactured by the following methods.

The first method for producing the electrode comprises a process for forming a layer for preventing noise electric wave comprising the thermal sprayed layer which is formed on one surface of the electrode substrate, and in which thermal spraying is performed in the direction perpendicular to the surface, and which has the porosity of not more than 20%; and a process for removing the thermal sprayed layer in which thermal spraying is performed on the other surface of the electrode substrate, and which has the porosity of more than 20%.

In the first method for producing the electrode, the means for removing the thermal sprayed layer in which thermal spraying is performed on the other surface of the electrode substrate, and which has the porosity of more than 20% is not especially restricted. For example, a grinding processing by means of grinder can be used.

The second method for producing the electrode comprises a process for laminating a number of electrode substrates; a process for forming the layer for preventing noise electric wave comprising the thermal sprayed layer which is formed

on each edge surface of each electrode substrate, and in which thermal spraying is performed in the direction perpendicular to each edge surface, and which has the porosity of not more than 20%; and a process for separating the layer for preventing noise electric wave along a dividing line of each electrode substrate.

The third method for producing the electrode comprises a process for laminating a number of electrode substrates having a spacer therebetween in which edge portion of each spacer is projected from the edge surface of each electrode substrate by the predetermined length; a process for forming the layer for preventing noise electric wave comprising the thermal sprayed layer which is formed on each edge surface of each electrode substrate, and in which thermal spraying is performed in the direction perpendicular to each edge surface in such a manner that the thickness of the thermal sprayed layer is thinner than the above predetermined length, and which has the porosity of not more than 20%; and a process for removing the layer for preventing noise electric wave from each spacer.

The fourth method for producing the electrode comprises a process for laminating a number of electrode substrates; a process for forming the substrate thermal sprayed layer which is formed on each edge surface of each electrode substrate, and in which thermal spraying is performed in the direction perpendicular to each edge surface; a process for separating the substrate thermal sprayed layer along a dividing line of each electrode substrate; a process for re-laminating each electrode substrate coated with the substrate thermal sprayed layer; a process for forming the layer for preventing noise electric wave comprising the thermal sprayed layer which is coated on the substrate thermal sprayed layer formed on each edge surface of each electrode substrate, and in which thermal spraying is performed in the direction perpendicular to each edge surface of re-laminating electrode substrate, and which has the porosity of not more than 20%; and a process for separating the layer for preventing noise electric wave along a dividing line of each electrode substrate.

In the second to fourth methods, it is preferable that the layer for preventing noise electric wave is made a notch by cutter or grinder for cutter to be separated.

The fifth method for producing electrode comprises a process for laminating a number of electrode substrates; a process for forming the layer for preventing noise electric wave comprising the thermal sprayed layer which is formed on each edge surface of each electrode substrate, and in which thermal spraying is performed in the direction perpendicular to each edge surface in such a manner that the electrode substrate is swung in order to repeat relative displacement between the two edge surfaces of two neighboring electrode substrates, and which has the porosity of not more than 20%.

In the second to fifth methods, it is preferable that a number of electrode substrates are laminated in such a manner that each edge surface of each electrode substrate faced to the opposite electrode is exposed on the same surface because it is necessary to form the layer for preventing noise electric wave on the edge surface of the electrode substrate faced to the opposite electrode.

In the second to fifth methods, it is preferable that the electrode substrates having wide area are laminated with each other since the thermal spraying materials are not adhered to the surface of the electrode substrate which is horizontal to the thermal spraying direction. Namely, when the edge surface of the electrode substrates is rectangular

form, it is preferable that the electrode substrates are laminated with each other in such a manner that the surface having long edge is overlapped with the other surface having long edge. It is more preferable that the electrode substrate is laminated with each other not only in one direction but also in two crossing directions in order that the thermal spraying materials are not adhered to the surface which is horizontal to the thermal spraying direction.

The sixth method for producing the electrode comprises a process for forming the layer for preventing noise electric wave comprising the thermal sprayed layer which is formed on one surface of long-shaped electrode substrate, and in which thermal spraying is performed in the direction perpendicular to the surface and which has the porosity of not more than 20%; and a process for separating the long-shaped electrode substrates into many pieces.

In the second to sixth methods, it is preferable that the porous thermal sprayed layer in which the thermal spraying materials are adhered to the surface which is horizontal to the thermal spraying direction is removed by grinding processing or fused by high density energy to be densified as mentioned thereafter.

The seventh method for producing the electrode comprises a process for forming a layer for preventing noise electric wave comprising the thermal sprayed layer which is formed on one surface of the electrode substrate, and in which thermal spraying is performed in the direction perpendicular to the surface, and which has the porosity of not more than 20%; and a process for fusing the thermal sprayed layer in which thermal spraying is performed on the other surface of the electrode substrate, and which has the porosity of more than 20% by means of high density energy to be densified.

In the first to seventh methods, when the thermal spraying is performed on the surface of the electrode substrate in the approximately perpendicular direction, the thermal spraying condition is not especially restricted if only the porosity of the thermal sprayed layer is not more than 20%.

The electrode for preventing noise electric wave for solving the above first and third objects comprises a substrate; a high-fusing conductive material layer which is formed on the surface of the substrate faced to the opposite electrode, and which has the resistivity of not more than  $10^4$  ohm centimeters, the fusing point of not less than  $2000^\circ\text{C}$ ., and the thickness of not more than 30 micron seconds; and not less than one resisting material layer which is coated on the surface of the high-fusing conductive material layer faced to the opposite electrode.

The following is the reason that the resistivity, the fusing point, and the thickness of the high-fusing conductive material layer are restricted.

When the resistivity of the high-fusing conductive material layer is larger than  $10^4$  ohm centimeters, the discharge portion is moved to the side of the substrate. As a result, the concave portion is generated at the portion of the substrate which is near the boundary portion between the substrate and the high-fusing conductive material layer due to fused loss so that the performance is deteriorated. It is defined that the resistivity is always measured at the temperature of  $20^\circ\text{C}$ .

When the fusing point of the high-fusing conductive material layer is less than  $2000^\circ\text{C}$ ., it is possible that the performance is deteriorated due to fused loss of the high-fusing conductive material layer itself. Furthermore, when the thickness of the high-fusing conductive material layer is less than 30 microns, the effect of the high-fusing conductive

material layer cannot be obtained, and the heat from the discharge portion is moved to the substrate. Therefore, the concave portion is generated at the portion of the substrate which is near the boundary portion between the substrate and the high-fusing conductive material layer due to fused loss.

Materials of the high-fusing conductive material layer is not specially restricted if only the materials can satisfy the above conditions. Therefore, the high-fusing conductive material layer comprises not less than one kind of materials consisting of Mo (having the resistivity of  $5.7 \times 10^{-6}$  ohm centimeters, and the fusing point of  $2622^\circ\text{C}$ .), Ta (having the resistivity of  $13.5 \times 10^{-6}$  ohm centimeters and the fusing point of  $2850^\circ\text{C}$ .), W (having the resistivity of  $5.5 \times 10^{-6}$  ohm centimeters and the fusing point of  $3382^\circ\text{C}$ .),  $\text{Cr}_2\text{O}_3$  (having the resistivity of 10 to  $10^2$  ohm centimeters and the fusing point of  $2270^\circ\text{C}$ .) and  $\text{CeO}_2$  (having the resistivity of  $10^3$  ohm centimeters and the fusing point of  $2660^\circ\text{C}$ .)

It is preferable that the substrate comprises copper or copper alloy. In the high-fusing conductive material layer, when the high density energy due to discharge is concentrated to accumulate heat, especially when the amount of accumulated heat increases at the time of high speed rotation, there is the possibility that the high-fusing conductive material layer is fused and damaged. Therefore, the substrate comprises copper or copper alloy having high heat conductivity so that outgoing radiation is promoted, thereby preventing the substrate from being fused and damaged.

Materials of the resisting material layer is not especially restricted. Therefore, the resisting material layer comprises an insulator of  $\text{Al}_2\text{O}_3$ ,  $\text{SiO}_2$ ,  $\text{ZrO}_2$ ,  $\text{MgO}$  and the like, or a mixture of the insulator and a resistor of  $\text{CuO}$ ,  $\text{Cr}_2\text{O}_3$ ,  $\text{NiO}$ ,  $\text{ZnO}$ ,  $\text{TiO}_2$  and the like.

The electrode for preventing noise electric wave for solving the above first and third objects comprises a substrate, a resisting material layer which is coated on the surface of the substrate faced to the opposite electrode. In this electrode, the substrate has a covering portion which is covered on the outer periphery of the resisting material layer and is located at the connecting portion between the substrate and the resisting material layer.

It is preferable that the shape of the covering portion of the substrate is circular form in order to cover the whole periphery of the resisting material layer. When the sectional form of the electrode is rectangular form in which the length of the long edge is remarkably longer than the length of the short edge, the covering portion can cover only the surfaces having wide area of the outer periphery of the resisting material layer.

It is preferable that the thickness of the covering portion of the substrate is not more than 0.34 mm. When the thickness of the covering portion is more than 0.34 mm, the covering portion is fused and damaged by the heat at the time of discharge. At the same time, the concave portion generated at the covering portion becomes deep, and noise electric wave becomes increasing.

The length of the covering portion of the substrate is determined in accordance with the endurance travel distance, but it is preferable that the length of the covering portion is not less than 0.1 mm. When the length of the covering portion is shorter than 0.1 mm, the covering portion is fused and damaged to be small. As a result, the discharge portion is generated from the substrate except the covering portion at the earlier stage so that the required performance cannot be obtained.

In the electrode for preventing noise electric wave, the material of the resisting material layer is the same as those

of the resisting material layer in the electrode for preventing noise electric wave.

(Effects)

In the electrode for preventing noise electric wave, the second layer which is located at outside has larger resistivity than that of the first layer.

When the discharge occurs, the flow of electron in the oxide resistor continuously exists for a predetermined time. However, when electron is once emitted, the electronic supply performance at the top surface layer has an enormous influence on the current value. As a result, it is advantageous that the impedance of the second layer is high. In the electrode having the above construction, it is possible to prevent the generation of noise electric wave as compared with the conventional electrode having single layer comprising high electrical resistance substance.

In the electrode for preventing noise electric wave, discharge is generated from the oxide resistor (having lower resistance than that of the oxide dielectric substance) in the first layer at the time of voltage apply, but the oxide dielectric substance exists in the second layer. Therefore, discharge is generated from the upper and lower surfaces of the electrode, and current flows along the surface of the first and second layers to be creeping discharge. When electron is moved along the surface of the first and second layers having high electric resistance, energy of the discharge is damped and the generation of the electric field and magnetic field which causes noise can be decreased. Furthermore, since the second layer comprising oxide dielectric substance is formed on the first layer, the outflow of electron charged in the oxide resistor in the first layer can be prevented when the electron of the creeping discharge is moved from the electrode for preventing noise electric wave (cathode) to the opposite electrode (anode). When the outflow of electron charged in the oxide resistor in the first layer occurs, discharge current value is increased and noise electric wave is increased.

In the electrode for preventing noise electric wave, when the second layer comprising oxide dielectric substance is too thick, impedance of whole electrode is increased and discharge voltage is increased. As a result, the effect for preventing noise electric wave is deteriorated. Therefore, it is preferable that the thickness of the second layer is not more than 0.1 mm. In order to effectively demonstrate the effect of the above creeping discharge, the total thickness of the first layer and the second layer is in the range of 0.1 to 1.0 mm. When the total thickness of the first layer and the second layer is not less than 1.0 mm, impedance of whole electrode is increased. Furthermore, discharge is generated at the oxide resistor in the first layer from which discharge is likely to be generated, and at the field which is nearest to the opposite electrode. Namely, discharge is generated from the boundary portion between the first layer and the second layer, thereby deteriorating the effect of creeping discharge.

The electrode of the present invention is exposed to the high density energy due to the discharge. In the electrode, when the oxide dielectric substance of the second layer is used as a barrier for saving the discharge electron, large amounts of energy is absorbed, and the electrode sectionally becomes high temperature. As a result, when the oxide resistor having comparatively low fusing point such as CuO is used for the first layer, the oxide resistor are fused by the heat. Furthermore, when the electrode rotates at high speed like a rotor, the oxide dielectric substance of the second layer is also scattered to generate pin hole.

To prevent the above disadvantages, the oxide dielectric substance and the oxide resistor have preferably high fusing

point. Inventors have found that the temperature at the time of discharge reaches 1300° to 1500° C. sectionally. Therefore, the oxide dielectric substance and the oxide resistor have preferably the fusing point of not less than 1500° C. The oxide dielectric substances include  $Al_2O_3$ ,  $ZrO_2$ ,  $MgO$ ,  $BeO$  and so on. The oxide resistors include  $TiO_2$ ,  $CaO$ ,  $MnO$ ,  $ZnO$ ,  $BaO$ ,  $CeO_2$ ,  $NiO$ ,  $CoO$ ,  $Fe_3O_4$ ,  $Cr_2O_3$ ,  $V_2O_3$  and so on.

However, in the case of the above composition, the pin hole is sometimes generated. So, in the electrode for firmly preventing the pin hole, the second layer comprises both the oxide dielectric substance and the oxide resistor. As a result, the resistivity value of the second layer is decreased as compared with the electrode. Furthermore, the performance of the barrier is deteriorated, and the absorbed energy can be decreased. Therefore, sectionally temperature rising of the electrode can be controlled, and it is possible to prevent the fusion of the resistor and the dielectric substance which causes the generation of the pin hole.

In the present invention, oxide is used for the resistor or the dielectric substance. When carbide or nitride is used for the resistor or the dielectric substance, the discharge in the atmosphere causes the deterioration of oxidation, and there are disadvantages in the durability of the performance for preventing noise electric wave.

In the electrodes of the present invention, it is preferable that the thickness of the first layer is in the range of 0.1 to 1.0 mm, and the total thickness of the first layer and the second layer is not more than 1.0 mm. When the thickness of the first layer is less than 0.1 mm, it is difficult to decrease the discharge voltage. When the total thickness of the first layer and the second layer is more than 1.0 mm, it is easy to cause coming-off or loss of the layer. In case of the rotor electrode, there are bad influence on the performance of the ignition of engine. Furthermore, in the described electrode, the effect of creeping discharge is deteriorated.

In the electrode for preventing noise electric wave, the second layer is formed on the surface of the first layer by performing oxidation treatment on the surface of the first layer. Therefore, this method has advantages in the cost as compared with plasma spraying method, ion plating method, sputtering method and so on.

In the electrodes for preventing noise electric wave, the layer for preventing noise electric wave comprising thermal sprayed layer is coated on the surface of the electrode substrate faced to the opposite electrode and has the porosity of not more than 20%. Therefore, the generation of the micro discharge at the porous portion of the thermal sprayed layer, which induces the induction discharge current having comparatively high absolute value level of the current value at the time of discharge to flow for a long time, can be controlled.

In the first method for producing the electrode, since the layer for preventing noise electric wave comprising the thermal sprayed layer and having the porosity of not more than 20% is confirmly formed only on the surface of the electrode substrate faced to the opposite electrode, it is possible to provide the electrode for preventing noise electric wave which can firmly prevent the generation of the micro discharge at the porous portion of the thermal sprayed layer.

In the second to fifth methods for producing the electrode, since thermal spraying is performed at each edge surface of a number of laminated electrode substrates, it is possible to prevent the formation of the porous thermal sprayed layer at least on the overlapping surface made by two neighboring electrode substrates. At the same time, it is possible to manufacture many electrodes productively.

In the third method for producing the electrode, the edge portion of each spacer located between laminated electrode substrates is projected from the edge surface of each electrode substrate by the predetermined length, and at the same time, thermal spraying is performed in such a manner that the thickness of the thermal sprayed layer is thinner than the above predetermined length. As a result, each layer for preventing noise electric wave formed on each electrode substrate is previously separated by each spacer. Therefore, it is possible to control coming-off of the layer at the time of separating the layer for preventing noise electric wave.

In the fourth method for producing the electrode, the substrate thermal spraying layer formed on the edge surface of each of the laminated electrode substrate is separated along a dividing line of electrode substrate, and then each electrode substrate is re-laminated. After that, the layer for preventing noise electric wave is formed on the separated substrate thermal spraying layer. As a result, when the layer for preventing noise electric wave is separated along the dividing line of each electrode substrate, a breaking portion of the substrate thermal spraying layer is the stress concentration point. Therefore, the layer for preventing noise electric wave is easily and firmly separated by the breaking portion.

In the fifth method for producing the electrode, thermal spraying is performed, and at the same time, the electrode substrate is swung in order to repeat relative displacement between two edge surfaces of two neighboring electrode substrates. As a result, the layer for preventing noise electric wave formed on each electrode substrate is not adhered to each other. Therefore, it is possible to omit the process for separating the layer for preventing noise electric wave, and to prevent coming-off of the layer in the process for separating the layer.

In the sixth method for producing the electrode, the layer for preventing noise electric wave is formed on one surface of long-shaped electrode substrate, and then the layer for preventing noise electric wave is cut into many pieces. Therefore, it is possible to prevent the formation of the porous thermal sprayed layer at least on the cut surface of each electrode substrate, and to manufacture many electrodes productively. Furthermore, it is possible to prevent coming-off or slippage of the layer since the layer for preventing noise electric wave is cut by machining.

In the seventh method for producing the electrode, the porous thermal sprayed layer formed on the surface of the electrode substrate which is horizontal to the thermal spraying direction is fused by high density energy to be densified, and the porous portion of the thermal sprayed layer is firmly omitted. Therefore, it is possible to provide the electrode for preventing noise electric wave which can firmly prevent the generation of the micro discharge at the porous portion of the thermal sprayed layer.

In the electrode for preventing noise electric wave, the high-fusing conductive material layer having special resistivity, fusing point and thickness exists between the substrate and the resisting material layer. As a result, since discharge is generated from the high-fusing conductive material layer, not from the substrate, the substrate having comparatively low fusing point is hardly fused and damaged by the heat at the time of discharge. Therefore, it is possible to prevent the formation of the concave portion which causes the increase in noise electric wave on the surface of the substrate. Furthermore, since the high-fusing conductive material layer has high fusing point, the high-fusing conductive material is hardly fused and damaged by the heat, and the concave portion is hardly formed on the high-fusing conductive material layer.

When the substrate comprises copper or copper alloy having high heat conductivity, the radiation effect from the substrate can be obtained since copper or copper alloy has high heat conductivity. Therefore, it is possible to control the concentration of the high density energy due to discharge at the high-fusing conductive material layer, and to decrease the possibility that the high-fusing conductive material layer is fused and damaged.

In the electrode for preventing noise electric wave, the substrate has the covering portion which is covered on the outer periphery of the resisting material layer and is located at the connecting portion between the substrate and the resisting material layer. At the portion of the covering portion which is near a boundary portion between the tip portion of the covering portion and the resisting material layer, discharge is generated. At this time, the covering portion is fused and damaged by the heat at the time of discharge, but the resisting material layer located at the lower surface of the covering portion is less fused and damaged since the resisting material has higher fusing point than that of the base material. Therefore, the damage of fused loss which causes the increase in noise electric wave is checked by the thickness of the covering portion, and the concave portion is hardly formed at the resisting material layer.

When the thickness of the covering portion of the substrate is not more than 0.34 mm, noise electric wave is hardly increased due to the influence of fused loss on the covering portion which is caused by the heat at the time of discharge.

When the coating portion of the substrate is not less than 0.1 mm, it is possible to extend the period that discharge is generated from the substrate except the coating portion which becomes gradually small. Therefore, it is possible to improve the durability.

#### BRIEF DESCRIPTION OF THE DRAWINGS

A more complete appreciation of the present invention and many of its advantages will be readily obtained as the same becomes better understood by reference to the following detailed description when considered in connection with the accompanying drawings and detailed specification, all of which forms a part of the disclosure:

FIG. 1 is a main cross-sectional view for showing the electrode for preventing noise electric wave according to the First Preferred Embodiment of the present invention.

FIG. 2 is a whole cross-sectional view for showing the electrode for preventing noise electric wave according to the First Preferred Embodiment of the present invention.

FIG. 3 is a bar graph for showing the level of noise electric wave of the electrode according to the First Preferred Embodiment of the present invention.

FIG. 4 is a graph for showing the relationship between the level of noise electric wave and the ratio of the resistivity of the second layer to the resistivity of the first layer according to the First Preferred Embodiment of the present invention.

FIG. 5 is a graph for showing the degree of the discharge voltage of the electrode according to the Second Preferred Embodiment of the present invention.

FIG. 6 is a graph for showing the degree of the noise electric current of the electrode according to the Second Preferred Embodiment of the present invention.

FIG. 7 is a graph for showing the degree of the noise electric field intensity of the electrode according to the Second Preferred Embodiment of the present invention.

FIG. 8 is an enlarged photograph for showing the particle structure on the surface of the second layer of the electrode

according to the Second Preferred Embodiment of the present invention after the electrode is used.

FIG. 9 is a bar graph for showing the level of noise electric wave of the electrode according to the Third Preferred Embodiment of the present invention.

FIG. 10 is a graph for showing the relationship between the level of noise electric wave and the thickness of the first layer according to the Third Preferred Embodiment of the present invention.

FIG. 11 is a graph for showing the relationship between the level of noise electric wave and the thickness of the second layer according to the Third Preferred Embodiment of the present invention.

FIG. 12 is a bar graph for showing the level of noise electric wave of the electrode according to the Fourth Preferred Embodiment of the present invention.

FIG. 13 is a graph for showing the relationship between the level of noise electric wave and the amount of  $TiO_2$  according to the Fourth Preferred Embodiment of the present invention.

FIG. 14 is a graph for showing the relationship between the level of noise electric wave and the thickness of the first layer according to the Fourth Preferred Embodiment of the present invention.

FIG. 15 is a whole cross-sectional view for showing the electrode for preventing noise electric wave according to the Fifth Preferred Embodiment of the present invention.

FIG. 16 is a main cross-sectional view for showing the electrode for preventing noise electric wave according to the Fifth Preferred Embodiment of the present invention.

FIG. 17 is a cross-sectional view for explaining the method for producing the electrode according to the Embodiment 26.

FIG. 18 is a graph for showing the relationship among the porosity of the thermal sprayed layer, PNL operating time and the radiation electric field intensity according to the Embodiment 26.

FIG. 19 is a graph for showing the relationship among the thickness of the porous thermal sprayed layer, PNL operating time and the radiation electric field intensity according to the Embodiment 26.

FIG. 20 is a main cross-sectional view for showing the electrode for preventing noise electric wave which is manufactured by the conventional method. FIG. 21 is a cross-sectional view for explaining the method for producing the electrode according to the Embodiment 27.

FIG. 22 is a cross-sectional view for showing the variations of the method for producing the electrode according to the Embodiment 28.

FIG. 23 is a cross-sectional view for explaining the method for producing the electrode according to the Embodiment 29.

FIG. 24 is a cross-sectional view for explaining the method for producing the electrode according to the Embodiment 30.

FIG. 25 is a plane view for showing the electrode substrate according to the Embodiment 31.

FIG. 26 is a cross-sectional view for explaining the method for producing the electrode according to the Embodiment 32.

FIG. 27 is a cross-sectional view along line A—A of FIG. 26 according to the Embodiment 32.

FIG. 28 is a cross-sectional view along line B—B of FIG. 26 according to the Embodiment 32.

FIG. 29 is a cross-sectional view along line C—C of FIG. 26 according to the Embodiment 32.

FIG. 30 is a graph for showing the relationship between the fraction defective of the thermal sprayed layer and the thickness of the thermal sprayed layer which is formed during 1 cycle of swing according to the Embodiment 32.

FIG. 31 is a graph for showing the relationship between the fraction defective of the thermal sprayed layer and the value of  $s$  (swing amplitude)/d (particle diameter after thermal spraying) according to the Embodiment 32.

FIG. 32 is a graph for showing the relationship among the porosity of the thermal sprayed layer formed on the surface of the electrode substrate which is parallel to the thermal spraying direction, PNL operating time and the radiation electric field intensity according to the Embodiment 33.

FIG. 33 is a graph for showing the result of examining PNL operating time and the induced discharge wave form before the porous thermal sprayed layer is fused by the high density energy.

FIG. 34 is a graph for showing the result of examining PNL operating time and the induced discharge wave form after the porous thermal sprayed layer is fused by the high density energy to be densified.

FIG. 35 is a whole cross-sectional view for showing the electrode for preventing noise electric wave according to the Sixth Preferred embodiment of the present invention.

FIG. 36 is a graph for showing the relationship between the endurance time and the level of noise electric wave according to the Sixth Preferred embodiment of the present invention.

FIG. 37 is a graph for showing the relationship between the thickness of the high-fusing conductive material layer and the level of noise electric wave according to the Sixth Preferred Embodiment of the present invention.

FIG. 38 is a whole cross-sectional view for showing the electrode for preventing noise electric wave according to the Seventh Preferred Embodiment of the present invention.

FIG. 39 is a graph for showing the relationship between the endurance time and the level of noise electric wave according to the Seventh Preferred Embodiment of the present invention.

FIG. 40 is a graph for showing the thickness of the coating portion and the level of noise electric wave according to the Seventh Preferred Embodiment of the present invention.

FIG. 41 is a bar graph for showing the level of noise electric wave of the electrode according to the Eighth Preferred Embodiment of the present invention.

FIG. 42 is a cross-sectional view for typically showing discharge generation situation according to the Eighth Preferred Embodiment of the present invention.

FIG. 43 is an enlarged cross-sectional view for typically showing discharge generation situation according to the Eighth Preferred Embodiment of the present invention.

FIG. 44 is a graph for showing the relationship between the thickness of the second layer and the level of noise electric wave according to the Eighth Preferred Embodiment of the present invention.

FIG. 45 is a graph for showing the result of examining the electric current profile model at the time of first discharge in the conventional electrode for preventing noise electric wave.

FIG. 46 is a graph for showing the result of comparison between the electric current profile model at the time of first discharge in the conventional electrode with the layer for

preventing noise electric wave and the electric current profile model at the time of first discharge in the conventional electrode without the layer.

#### DETAILED DESCRIPTION OF THE PREFERRED EMBODIMENTS

Having generally described the present invention, a further understanding can be obtained by reference to the specific preferred embodiment which is provided herein for purposes of illustration only and is not intended to limit the scope of the appended claims.

In the following preferred embodiments, the present invention is applied for a rotor electrode of distributor of automobiles. FIG. 2 is a whole schematic diagram of this electrode. The distributor comprises a rotor 1 which is rotatable at high speed, a rotor electrode 2 which is installed on the rotor 1 and a side electrode 3 which is opposite to the tip of the rotor electrode 2 with the clearance therebetween.

##### First Preferred Embodiment

###### Embodiment 1

FIG. 1 is a cross-sectional view for showing the rotor electrode 2 according to the Embodiment 1. The rotor electrode 2 comprises a substrate 20 made of brass, a substrate layer 21 formed on the surface of the substrate 20, a first layer 22 formed and coated on the surface of the substrate layer 21 and a second layer 23 formed and coated on the surface of the first layer 22.

The substrate layer 21 is formed in such a manner that the first layer 22 is firmly adhered to the substrate 20 by thermal spraying. The substrate layer 21 is made of Ni-5% Al alloy and has the thickness of 100 microns. The substrate layer 21 is formed by plasma spraying method.

The first layer 22 is made of CuO as oxide resistor and has the thickness of 200 microns. The resistivity value  $R_1$  of the first layer 22 is in the range of  $10^3$  to  $10^4$  ohm centimeters.

The second layer 23 is made of BaO as oxide resistor and has the thickness of 200 microns. The resistivity value  $R_2$  of the second layer 23 is in the range of  $10^9$  to  $10^{10}$  ohm centimeters. Therefore,  $R_2$  is larger than  $R_1$ .

Both the first layer 22 and the second layer 23 are formed by plasma spraying method.

###### Comparative Example 1

An electrode according to Comparative Example 1 comprises only a substrate 20.

###### Comparative Example 2

An electrode according to Comparative Example 2 has the same construction as that of the Embodiment 1 except that the second layer 23 is not existed.

###### Comparative Example 3

An electrode according to Comparative Example 3 has the same construction as that of the Embodiment 1 except that the first layer 22 formed on the surface of the substrate layer 21 is made of BaO and has the thickness of 200 microns, and that the second layer 23 is not existed.

###### Comparative Example 4

An electrode according to Comparative Example 4 has the same construction as that of the Embodiment 1 except that the first layer 22 formed on the surface of the substrate layer

21 is made of BaO and has the thickness of 200 microns, and that the second layer 23 is made of CuO and has the thickness of 200 microns. In this case, the resistivity value  $R_2$  of the second layer 23 is smaller than the resistivity value  $R_1$  of the first layer 22.  
(Evaluation)

FIG. 3 shows the result of measuring the level of noise electric wave at the time of discharge concerning each electrode. As seen from FIG. 3, the electrode according to the Embodiment 1 shows the most excellent effect for preventing noise electric wave. As seen from Comparative Example 4, when the first layer 22 and the second layer 23 in the Embodiment 1 are exchanged with each other, there is no effect for preventing noise electric wave.

FIG. 4 shows the change of the level of noise electric wave when the ratio of  $R_2$  to  $R_1$  ( $R_2/R_1$ ) is variously changed. As seen from FIG. 4, when  $R_1$  is larger than or equal to  $R_2$ , there is no effect for preventing noise electric wave. Furthermore, when  $R_2$  is larger than  $R_1$ , there is remarkable effect for preventing noise electric wave.

##### Second Preferred Embodiment

###### Embodiment 2

An electrode according to the Embodiment 2 has the same construction as that of the Embodiment 1 except that the construction of the first layer 22 and the second layer 23 is different. The first layer 22 is made of the mixture comprising  $Al_2O_3$  as oxide dielectric substance and CuO as oxide resistor, and the weight ratio of  $Al_2O_3$  to CuO is 4:6. The first layer 22 has the thickness of 400 microns, and the resistivity value is in the range of  $10^4$  to  $10^6$  ohm centimeters.

The second layer 23 is made of only  $Al_2O_3$  as oxide dielectric substance. The second layer 23 has the thickness of 50 microns, and the resistivity value is  $10^{14}$  ohm centimeters. The second layer 23 has the larger resistivity than that of the first layer 22.

Both the first layer 22 and the second layer 23 are formed by plasma spraying method which is the same method as that in the Embodiment 1.

###### Comparative Example 1

An electrode according to Comparative Example 1 comprises only a substrate 20.

###### Comparative Example 5

An electrode according to Comparative Example 5 has the same construction as that of the Embodiment 2 except that the second layer 23 is not existed.

###### Comparative Example 6

An electrode according to Comparative Example 6 has the same construction as that of the Embodiment 1 except that an insulation layer is formed on the surface of the substrate layer 21 in order to propagate electric power by use of creeping discharge. The insulation layer is made of  $Al_2O_3$  and has the thickness of 400 microns.  
(Evaluation)

Concerning each electrode, the discharge voltage, noise electric current and noise electric field intensity were measured. The result is shown in FIGS. 5, 6 and 7.

As seen from these figures, both the discharge voltage and noise electric current of the Embodiment 2 are controlled to be low. As a result, noise electric field intensity is remarkably decreased. As compared with Comparative Examples 5

17

and 6, the electrode of the Embodiment 2 has about 2.5 to 3 times effect for decreasing noise electric wave.

### Third Preferred Embodiment

#### Embodiment 3

When the electrode of Embodiment 2 is used, as shown in FIG. 8, a number of pin holes (circle and black portions) are generated on the surface of the second layer 23, and the effect for preventing noise electric wave is gradually decreased. Therefore, an electrode according to the Embodiment 3 has the same construction as that of the Embodiment 1 except that the first layer 22 is made of electromelting grinding material such as  $Al_2O_3$ -13%  $TiO_2$  (in case of not more than 44%  $TiO_2$ , it exists as  $Al_2TiO_5$  and  $Al_2O_3$ ) and has the thickness of 20 microns, and that the second layer is made of  $Al_2O_3$  and has the thickness of 50 microns.

The electromelting grinding material comprising  $Al_2O_3$ -13%  $TiO_2$  is now put on the market, and it is excellent in its uniformity of dispersion and the cost. When the electromelting grinding material is used as the first layer, it is possible to manufacture the electrode for preventing noise electric wave having excellent performance inexpensively.

#### Embodiment 4

An electrode according to the Embodiment 4 has the same construction as that of the Embodiment 3 except that the thickness of the first layer 22 is 70 microns.

#### Embodiment 5

An electrode according to the Embodiment 5 has the same construction as that of the Embodiment 3 except that the thickness of the first layer 22 is 100 microns.

#### Embodiment 6

An electrode according to the Embodiment 6 has the same construction as that of the Embodiment 3 except that the thickness of the first layer 22 is 200 microns.

#### Embodiment 7

An electrode according to the Embodiment 7 has the same construction as that of the Embodiment 3 except that the thickness of the first layer 22 is 800 microns.

#### Embodiment 8

An electrode according to the Embodiment 8 has the same construction as that of the Embodiment 3 except that the thickness of the first layer 22 is 400 microns, and that the thickness of the second layer 23 is 20 microns.

#### Embodiment 9

An electrode according to the Embodiment 9 has the same construction as that of the Embodiment 3 except that the thickness of the first layer 22 is 400 microns.

#### Embodiment 10

An electrode according to the Embodiment 10 has the same construction as that of the Embodiment 3 except that the thickness of the first layer 22 is 400 microns, and that the thickness of the second layer 23 is 100 microns.

#### Embodiment 11

An electrode according to the Embodiment 11 has the same construction as that of the Embodiment 3 except that

18

the thickness of the first layer 22 is 400 microns, and that the thickness of the second layer 23 is 200 microns.

### Embodiment 12

An electrode according to the Embodiment 12 has the same construction as that of the Embodiment 3 except that the thickness of the first layer 22 is 400 microns, and that the thickness of the second layer 23 is 400 microns.

### Comparative Example 1

An electrode according to Comparative Example 1 comprises only a substrate 20.

### Embodiment 13

An electrode according to the Embodiment 13 has the same construction as that of the Embodiment 3 except that the first layer 22 is made of the mixture comprising  $Al_2O_3$  and  $CuO$  (the weight ratio of  $Al_2O_3$  to  $CuO$  being 4 to 6) and has the thickness of 400 microns, and that the thickness of the second layer 23 is 100 microns.

### Embodiment 14

An electrode according to the Embodiment 14 has the same construction as that of the Embodiment 3 except that the first layer 22 is made of the mixture comprising  $Al_2O_3$  and  $CuO$  (the weight ratio of  $Al_2O_3$  to  $CuO$  being 4 to 6) and has the thickness of 400 microns, and that the thickness of the second layer 23 is 200 microns.

#### (Evaluation)

Concerning each electrode, the decreasing amount of the level of noise electric wave (decreasing amount of noise) having 180 MHz was measured at the initial stage and at 24 hours later. Furthermore, it was observed that the pin hole was generated or not after the electrode was used. The result is shown in Table 1 and FIG. 9. FIG. 10 shows the relationship between the thickness of the first layer 22 and the level of noise electric wave having 180 MHz, and FIG. 11 shows the relationship between the thickness of the second layer 23 and the level of noise electric wave having 180 MHz. The decreasing amount of noise is calculated on the basis of the initial performance of the electrode of Comparative Example 1.

The electrode according to the Embodiment 3 shows the low level of noise electric wave at the initial stage and at 24 hours later. On the contrary, the electrode according to the Embodiments 2 and 13 shows low level of noise electric wave at the initial stage, but noise electric wave becomes increasing at 24 hours later. This is caused by the generation of pin hole. When the second layer 23 is made of only  $Al_2O_3$  as oxide dielectric substance, pin hole is generated under the condition that  $CuO$  having comparatively low fusing point is included in the first layer 22.

In the Embodiment 14, no pin hole is generated and noise electric wave shows the same level at the initial stage and at 24 hours later. However, the level of noise electric wave is high since the thickness of the second layer 23 is thick. As seen from FIGS. 10 and 11, there is an appropriate thickness for preventing noise electric wave. The thickness of the first layer 22 is preferably not less than 0.1 mm, more preferably, not less than 0.2 mm. The thickness of the second layer 23 is preferably not more than 0.1 mm, more preferably, not more than 0.05 mm.

TABLE 1

|            | First Layer                                            |                | Second Layer                           |                | Decreasing Amount of Noise | Decreasing Amount of Noise | Generation  |
|------------|--------------------------------------------------------|----------------|----------------------------------------|----------------|----------------------------|----------------------------|-------------|
|            | Material                                               | Thickness (mm) | Material                               | Thickness (mm) | at Initial Stage (dB)      | after 24 Hours (dB)        | of Pin Hole |
| Com. Ex. 1 | —                                                      | —              | —                                      | —              | Standard                   | -2                         | —           |
| Embod. 2   | Al <sub>2</sub> O <sub>3</sub> + CuO                   | 0.4            | Al <sub>2</sub> O <sub>3</sub> (99.6%) | 0.05           | -26                        | -6                         | Yes         |
| Embod. 13  | Al <sub>2</sub> O <sub>3</sub> + CuO                   | 0.4            | Al <sub>2</sub> O <sub>3</sub> (99.6%) | 0.1            | -25                        | -8                         | Yes         |
| Embod. 14  | Al <sub>2</sub> O <sub>3</sub> + CuO                   | 0.4            | Al <sub>2</sub> O <sub>3</sub> (99.6%) | 0.2            | -10                        | -11                        | No          |
| Embod. 3   | Al <sub>2</sub> O <sub>3</sub> (13% TiO <sub>2</sub> ) | 0.02           | Al <sub>2</sub> O <sub>3</sub> (99.6%) | 0.5            | -10                        | -11                        | No          |
| Embod. 4   | Al <sub>2</sub> O <sub>3</sub> (13% TiO <sub>2</sub> ) | 0.07           | Al <sub>2</sub> O <sub>3</sub> (99.6%) | 0.05           | -11                        | -13                        | No          |
| Embod. 5   | Al <sub>2</sub> O <sub>3</sub> (13% TiO <sub>2</sub> ) | 0.1            | Al <sub>2</sub> O <sub>3</sub> (99.6%) | 0.05           | -16                        | -18                        | No          |
| Embod. 6   | Al <sub>2</sub> O <sub>3</sub> (13% TiO <sub>2</sub> ) | 0.2            | Al <sub>2</sub> O <sub>3</sub> (99.6%) | 0.05           | -24                        | -23                        | No          |
| Embod. 7   | Al <sub>2</sub> O <sub>3</sub> (13% TiO <sub>2</sub> ) | 0.8            | Al <sub>2</sub> O <sub>3</sub> (99.6%) | 0.05           | -28                        | -27                        | No          |
| Embod. 8   | Al <sub>2</sub> O <sub>3</sub> (13% TiO <sub>2</sub> ) | 0.4            | Al <sub>2</sub> O <sub>3</sub> (99.6%) | 0.02           | -25                        | -26                        | No          |
| Embod. 9   | Al <sub>2</sub> O <sub>3</sub> (13% TiO <sub>2</sub> ) | 0.4            | Al <sub>2</sub> O <sub>3</sub> (99.6%) | 0.05           | -27                        | -28                        | No          |
| Embod. 10  | Al <sub>2</sub> O <sub>3</sub> (13% TiO <sub>2</sub> ) | 0.4            | Al <sub>2</sub> O <sub>3</sub> (99.6%) | 0.11           | -16                        | -17                        | No          |
| Embod. 11  | Al <sub>2</sub> O <sub>3</sub> (13% TiO <sub>2</sub> ) | 0.4            | Al <sub>2</sub> O <sub>3</sub> (99.6%) | 0.2            | -10                        | -11                        | No          |
| Embod. 12  | Al <sub>2</sub> O <sub>3</sub> (13% TiO <sub>2</sub> ) | 0.4            | Al <sub>2</sub> O <sub>3</sub> (99.6%) | 0.4            | -11                        | -12                        | No          |

## Fourth Preferred Embodiment

## Embodiment 15

An electrode according to the Embodiment 15 has the same construction as that of the Embodiment 2 except that the second layer **23** is made of electromelting grinding material (Al<sub>2</sub>O<sub>3</sub>-2.3% TiO<sub>2</sub>) as semi-conductive alumina and has the thickness of 50 microns.

## Embodiment 16

An electrode according to the Embodiment 16 has the same construction as that of the Embodiment 15 except that the amount of TiO<sub>2</sub> in the second layer **23** is 5%.

## Embodiment 17

An electrode according to the Embodiment 17 has the same construction as that of the Embodiment 15 except that the thickness of the first layer **22** is 20 microns, and that the amount of TiO<sub>2</sub> in the second layer **23** is 13%.

## Embodiment 18

An electrode according to the Embodiment 18 has the same construction as that of the Embodiment 15 except that the thickness of the first layer **22** is 70 microns, and that the amount of TiO<sub>2</sub> in the second layer **23** is 13%.

## Embodiment 19

An electrode according to the Embodiment 19 has the same construction as that of the Embodiment 15 except that the thickness of the first layer **22** is 100 microns, and that the amount of TiO<sub>2</sub> in the second layer **23** is 13%.

## Embodiment 20

An electrode according to the Embodiment 20 has the same construction as that of the Embodiment 15 except that the amount of TiO<sub>2</sub> in the second layer **23** is 13%.

## Embodiment 21

An electrode according to the Embodiment 21 has the same construction as that of the Embodiment 15 except that the thickness of the first layer **22** is 800 microns, and that the amount of TiO<sub>2</sub> in the second layer **23** is 13%.

## Embodiment 22

An electrode according to the Embodiment 22 has the same construction as that of the Embodiment 15 except that the amount of TiO<sub>2</sub> in the second layer **23** is 30%.

## Embodiment 23

An electrode according to the Embodiment 23 has the same construction as that of the Embodiment 15 except that the amount of TiO<sub>2</sub> in the second layer **23** is 44%.

## Comparative Example 7

An electrode according to Comparative Example 7 has the same construction as that of the Embodiment 15 except that the second layer is made of 99% TiO<sub>2</sub>.

## Comparative Example 1

An electrode according to Comparative Example 1 comprises only a substrate **20**.

## Embodiment 2

An electrode according to the Embodiment 2 has the same construction as that of the Embodiment 1 except that the construction of the first layer **22** and the second layer **23** is different. The first layer **22** is made of the mixture comprising Al<sub>2</sub>O<sub>3</sub> as oxide dielectric substance and CuO as oxide resistor, and the weight ratio of Al<sub>2</sub>O<sub>3</sub> to CuO is 4:6. The first layer **22** has the thickness of 400 microns, and the direct current resistance value is in the range of 10<sup>4</sup> to 10<sup>6</sup> ohm centimeters.

The second layer **23** is made of only Al<sub>2</sub>O<sub>3</sub> as oxide dielectric substance. The second layer **23** has the thickness of 50 microns, and the direct current resistance value is 10<sup>14</sup> ohm centimeters. The direct current resistance value is measured instead of the resistivity, but the second layer **23** has the larger resistivity than that of the first layer **22**.

## Embodiment 13

An electrode according to the Embodiment 13 has the same construction as that of the Embodiment 2 except that the thickness of the second layer **23** is 100 microns.

## Embodiment 14

An electrode according to the Embodiment 14 has the same construction as that of the Embodiment 2 except that the thickness of the second layer **23** is 200 microns.

## 21

## Embodiment 25

An electrode according to the Embodiment 25 has the same construction as that of the Embodiment 2 except that the thickness of the second layer **23** is 20 microns. (Evaluation)

Concerning each electrode, the decreasing amount of the level of noise electric wave (decreasing amount of noise) having 180 MHz was measured at the initial stage and at 24 hours later. Furthermore, it was observed that the pin hole was generated or not after the electrode was used. The result is shown in Table 2 and FIG. 12. FIG. 13 shows the relationship between the added amount of  $TiO_2$  to the second layer **23** and the level of noise electric wave having 180 MHz, and FIG. 14 shows the relationship between the thickness of the first layer **22** and the level of noise electric wave having 180 MHz. The decreasing amount of noise is calculated on the basis of the initial performance of the electrode of Comparative Example 1.

The electrode according to the Embodiment 20 shows the low level of noise electric wave at the initial stage and at 24 hours later. On the contrary, the electrode according to the Embodiments 2, 13 and 25 shows low level of noise electric wave at the initial stage, but noise electric wave becomes increasing at 24 hours later. This is caused by the generation of pin hole. Although the first layer **22** includes  $CuO$  having comparatively low fusing point, pin hole is hardly generated when the second layer **23** is made of  $Al_2O_3$  as oxide dielectric substance and  $TiO_2$  as oxide resistor.

In the Embodiment 14, no pin hole is generated and noise electric wave shows the same level at the initial stage and at 24 hours later. However, the level of noise electric wave is high since the thickness of the second layer **23** is thick. As seen from FIGS. 13 and 14, there is an appropriate thickness of the first layer **22** and an appropriate added amount of  $TiO_2$  for preventing noise electric wave. The added amount of  $TiO_2$  is preferably in the range of 5 to 44%, more preferably, in the range of 5 to 22%. Furthermore, it is preferable that the thickness of the first layer is not less than 0.1 mm, more preferably, not less than 0.4 mm.

## 22

which is disposed at the rotor **1**, and a side electrode **3** which is faced to the tip of the rotor electrode **2** with the clearance therebetween. A layer **2a** for preventing noise electric wave comprising a thermal sprayed layer which is coated by 5 thermal spraying is formed on the edge surface of the rotor electrode **2** which is faced to the side electrode **3**.

## Embodiment 26

In the Embodiment 26, a rotor electrode **2** as the electrode 10 for preventing noise electric wave is manufactured by the first method according to claim 7.

As shown in the cross-sectional view of FIG. 16, the rotor electrode **2** according to the Embodiment 26 is made of brass having the thickness of 1.6 mm. The rotor electrode **2** 15 comprises an electrode substrate **20** which has two stepped portions **20a** and **20a** having each depth of about 1.2 mm and an edge surface **24**, and a layer **2a** for preventing noise electric wave comprising a thermal sprayed layer which is coated on the edge surface **24** by thermal spraying. The layer **2a** for preventing noise electric wave comprises 60 wt % of  $CuO$  and 40 wt % of  $Al_2O_3$ , and it has the porosity of 5% and the thickness of 400 microns.

The rotor electrode **2** is manufactured as follows. As 25 shown in FIG. 17, a number of the above electrode substrates **20** are laminated in such a manner that the edge surface **24** is uniform surface, and the laminated electrode substrates **20** are set in a tool (not shown). The tool covers the right and left side surfaces of each laminated electrode substrate **20**, the upper surface of the electrode substrate **20** 30 at the top and the lower surface of the electrode substrate **20** at the bottom. Then,  $Al_2O_3$ -60 wt %  $CuO$  material is thermal sprayed by plasma method in the direction which is perpendicular to the edge surface **24** of each electrode **20**. The thermal spraying by plasma method is performed under the condition that the porosity is set to be 5%, the voltage is 500V, the current is 75 A, the thermal spraying distance is 100 mm and the amount of powder supply is 40 g/minute. At this time, the thermal sprayed layer formed on the stepped portion **20a** of each electrode substrate **20** is not 35

TABLE 2

|            | First Layer     |                | Second Layer           |                | Decreasing Amount of Noise at Initial Stage (dB) | Decreasing Amount of Noise after 24 Hours (dB) | Generation of Pin Hole |
|------------|-----------------|----------------|------------------------|----------------|--------------------------------------------------|------------------------------------------------|------------------------|
|            | Material        | Thickness (mm) | Material               | Thickness (mm) |                                                  |                                                |                        |
| Com. Ex. 1 | —               | —              | —                      | —              | Standard                                         | -2                                             | —                      |
| Embod. 25  | $Al_2O_3 + CuO$ | 0.4            | $Al_2O_3(99.6\%)$      | 0.02           | -24                                              | -7                                             | Yes                    |
| Embod. 2   | $Al_2O_3 + CuO$ | 0.4            | $Al_2O_3(99.6\%)$      | 0.05           | -26                                              | -6                                             | Yes                    |
| Embod. 13  | $Al_2O_3 + CuO$ | 0.4            | $Al_2O_3(99.6\%)$      | 0.1            | -25                                              | -8                                             | Yes                    |
| Embod. 14  | $Al_2O_3 + CuO$ | 0.4            | $Al_2O_3(99.6\%)$      | 0.2            | -10                                              | -11                                            | No                     |
| Embod. 15  | $Al_2O_3 + CuO$ | 0.4            | $Al_2O_3(2.3\% TiO_2)$ | 0.05           | -25                                              | -13                                            | Yes                    |
| Embod. 16  | $Al_2O_3 + CuO$ | 0.4            | $Al_2O_3(5\% TiO_2)$   | 0.05           | -23                                              | -21                                            | No                     |
| Embod. 17  | $Al_2O_3 + CuO$ | 0.02           | $Al_2O_3(13\% TiO_2)$  | 0.05           | -11                                              | -13                                            | No                     |
| Ewbd. 18   | $Al_2O_3 + CuO$ | 0.07           | $Al_2O_3(13\% TiO_2)$  | 0.05           | -13                                              | -16                                            | No                     |
| Embod. 19  | $Al_2O_3 + CuO$ | 0.1            | $Al_2O_3(13\% TiO_2)$  | 0.05           | -16                                              | -18                                            | No                     |
| Embod. 20  | $Al_2O_3 + CuO$ | 0.4            | $Al_2O_3(13\% TiO_2)$  | 0.05           | -24                                              | -25                                            | No                     |
| Embod. 21  | $Al_2O_3 + CuO$ | 0.8            | $Al_2O_3(13\% TiO_2)$  | 0.05           | -24                                              | -25                                            | No                     |
| Embod. 22  | $Al_2O_3 + CuO$ | 0.4            | $Al_2O_3(30\% TiO_2)$  | 0.05           | -21                                              | -22                                            | No                     |
| Embod. 23  | $Al_2O_3 + CuO$ | 0.4            | $Al_2O_3(44\% TiO_2)$  | 0.05           | -16                                              | -19                                            | No                     |
| Com. Ex. 7 | $Al_2O_3 + CuO$ | 0.4            | $TiO_2(99\%)$          | 0.05           | -11                                              | -14                                            | No                     |

## Fifth Preferred Embodiment

As shown in FIG. 15, the distributor according to the Fifth Preferred Embodiment comprises a rotor **1** which is rotatable at high speed, a T-shaped and planar rotor electrode **2**

65 brought into contact with each other. Then, the tool is removed and each electrode substrate is disassembled. And, a grinding machining is performed in such a manner that a grinder is brought into contact with the stepped portion **20a**

## 23

of each electrode substrate **20**. Thus, the thermal sprayed layer formed on the stepped portion **20a** is removed and the rotor electrode **2** according to the Embodiment 26 is completed.

According to the Embodiment 26, the layer **2a** for preventing noise electric wave comprising the thermal sprayed layer having the porosity of not more than 20% is firmly formed only on the edge surface **24** of the electrode substrate **20**. Therefore, it is possible to provide the electrode for preventing noise electric wave which can firmly prevent the generation of micro discharge at the porous portion of the thermal sprayed layer.

(Relationship between the porosity of the layer for preventing noise electric wave and the effect for decreasing radio noise)

In the method according to the Embodiment 26, the thermal spraying distance at the time of thermal spraying by plasma method is changed, and the porosity of the layer **2a** for preventing noise electric wave is variously changed in the range of 5 to 50%, thereby manufacturing each rotor electrode. Concerning these rotor electrodes and the above completed rotor electrode **2**, PNL operating time and radiation electric field intensity were measured. The PNL operating time was measured by the turbulent time which is caused by that the positive magnetic wave is introduced from the radio antenna. At the same time, the radiation electric field intensity was measured by vehicles. The result is shown in FIG. 18.

As shown in FIG. 18, the PNL operating time becomes short as the porosity of the layer **2a** for preventing noise electric wave is decreased. When the porosity is decreased to be 20%, the decreasing rate becomes almost constant. The radiation electric field intensity maintains a certain value without receiving the influence of the porosity of the layer **2a** for preventing noise electric wave. As a result, when the porosity of the layer **2a** for preventing noise electric wave is set to be not more than 20%, the PNL operating time is drastically decreased. Therefore, it is possible to decrease the radio noise without decreasing the effect for preventing noise electric wave.

(Relationship between the thickness of the porous thermal sprayed layer and the effect for decreasing radio noise)

In the method according to Embodiment 26, the amount of grinding of the grinding machining is controlled, and the thickness **1** of the thermal sprayed layer formed on the stepped portion **20a** of the electrode substrate **20** is variously changed in the range of 0 to 200 microns, thereby manufacturing each rotor electrode. Concerning these rotor electrodes and the above completed rotor electrode **2**, PNL operating time and radiation electric field intensity were measured. The result is shown in FIG. 19. As shown in FIG. 20, the thickness **1** of the thermal sprayed layer formed on the stepped portion **20a** of the electrode substrate **20** is the maximum thickness, and the porosity of the thermal sprayed layer is about 50%. The thermal sprayed layer formed on the edge surface **24** of the electrode substrate has the thickness **L** of 400 microns, and the porosity of about 5%.

As shown in FIG. 19, the PNL operating time becomes short as the thickness of the porous thermal sprayed layer is decreased. When the porous thermal sprayed layer is completely removed, the PNL operating time becomes the shortest. The radiation electric field intensity maintains a certain value without receiving the influence of thickness of the porous thermal sprayed layer. As a result, when the thickness of the porous thermal sprayed layer becomes thin, the PNL operating time is decreased. Therefore, it is possible to decrease the radio noise without decreasing the effect for preventing noise electric wave.

## 24

## Embodiment 27

In the Embodiment 27, a rotor electrode **2** as the electrode for preventing noise electric wave is manufactured by the second method according to claim 8. The materials for the electrode substrate **20** and the layer **2a** for preventing noise electric wave are the same as those of the Embodiment 26, and the layer **2a** for preventing noise electric wave has the porosity of 5% and the thickness of 400 microns.

As shown in FIG. 21, a number of the electrode substrates **20** having the same thickness (1.6 mm) each other are laminated in such a manner that the edge surface **24** is uniform surface, and the laminated electrode substrates **20** are set in a tool (not shown). Then,  $\text{Al}_2\text{O}_3$ -60 wt % CuO material is thermal sprayed by plasma method in the direction which is perpendicular to the edge surface **24** of each electrode **20**. The thermal spraying by plasma method is performed under the same condition as that of the Embodiment 26. After the tool is removed, the layer **2a** for preventing noise electric wave is separated along a dividing line of each electrode substrate **20**. Thus, the rotor electrode **2** according to the Embodiment 27 is completed.

In the method according to Embodiment 27, the thermal spraying is performed to each edge surface **24** of many laminated electrode substrates **20**. Therefore, it is possible to prevent the formation of the porous thermal sprayed layer at least on the overlapping surface of the neighboring electrode substrates **20**. Furthermore, it is possible to manufacture many electrodes productively.

In order to prevent the coming-off of the layer at the time of separating the layer **2a** for preventing noise electric wave, it is preferable that the thickness of the layer **2a** is not more than 500 microns.

## Embodiment 28

In the Embodiment 28, a rotor electrode **2** is manufactured by the same method and same manners as those of the Embodiment 27 except the following. As shown in FIG. 22, after thermal spraying, the layer **2a** for preventing noise electric wave and the electrode substrate **20** are made a notch along the overlapped portion of the electrode substrate **20** by grinder for cutter (the thickness of 0.5 mm). The depth of the notch is twice as much as the thickness of the layer **2a** for preventing noise electric wave. Therefore, it is possible to easily and firmly separate the layer **2a** for preventing noise electric wave.

## Embodiment 29

In the Embodiment 29, a rotor electrode **2** as the electrode for preventing noise electric wave is manufactured by the third method according to claim 9. The materials for the electrode substrate **20** and the layer **2a** for preventing noise electric wave are the same as those of the Embodiment 26, and the layer **2a** for preventing noise electric wave has the porosity of 5% and the thickness of 400 microns.

A planar spacer **8** made of steel material having the thickness of 0.1 mm is prepared. As shown in FIG. 23, a number of the electrode substrates **20** having the same thickness (1.6 mm) each other and a number of spacers **8** are laminated in such a manner that the edge surface **24** is uniform surface and that the tip of each spacer **8** is projected from the edge surface **24** of the electrode substrate **20** by 1.0 mm, and the laminated electrode substrates **20** are set in a tool (not shown). The spacer **8** is disposed at the top and bottom edges in the laminated direction. Then,  $\text{Al}_2\text{O}_3$ -60 wt % CuO material is thermal sprayed by plasma method in the

## 25

direction which is perpendicular to the edge surface **24** of each electrode **20**. The thermal spraying by plasma method is performed under the same condition as that of the Embodiment 26. After the tool is removed, the layer **2a** for preventing noise electric wave is tore off from each spacer **8**. Thus, the rotor electrode **2** according to the Embodiment 29 is completed.

In the method according to Embodiment 29, the layer **2a** for preventing noise electric wave formed at the edge surface **24** of each electrode substrate **20** is previously separated by each spacer **8**. Therefore, it is possible to control the coming-off of the layer at the time of separating the layer **2a** for preventing noise electric wave.

The thickness of the spacer **8** is not especially restricted. However, it is necessary that the length **T** of the spacer **8** projected from the edge surface **24** is longer than at least the thickness **t** of the layer **2a** for preventing noise electric wave. It is preferable that the material of the spacer **8** is excellent in coming-off from the thermal sprayed material.

## Embodiment 30

In the Embodiment 30, a rotor electrode **2** as the electrode for preventing noise electric wave is manufactured by the fourth method according to claim 10. The materials for the electrode substrate **20** and the layer **2a** for preventing noise electric wave are the same as those of the Embodiment 26, and the layer **2a** for preventing noise electric wave has the porosity of 5% and the thickness of 400 microns.

As shown in FIG. 24, a number of the electrode substrates **20** having the same thickness (1.6 mm) each other are laminated in such a manner that the edge surface **24** is uniform surface, and the laminated electrode substrates **20** are set in a tool (not shown). Then, Ni-5% Al alloy as the thermal spraying material is thermal sprayed in the direction which is perpendicular to the edge surface **24** of each electrode **20** to form a substrate thermal sprayed layer **2b** having the thickness of 100 microns. After the tool is removed, the substrate thermal sprayed layer **2b** is separated along a dividing line of each electrode substrate **20**. Each electrode substrate **20** on which the substrate thermal sprayed layer **2b** is formed is re-laminated, and the re-laminated electrode substrates **20** are set in the tool. Then,  $\text{Al}_2\text{O}_3$ -60 wt % CuO material is thermal sprayed by plasma method in the direction which is perpendicular to the edge surface **24** of each electrode **20**. The thermal spraying by plasma method is performed under the same condition as that of the Embodiment 26. After the tool is removed, the layer **2a** for preventing noise electric wave is separated along a dividing line of each electrode substrate **20**. Thus, the rotor electrode **2** according to the Embodiment 30 is completed.

In the method according to Embodiment 30, when the layer **2a** for preventing noise electric wave is separated along each electrode substrate **20**, a breaking portion of the substrate thermal sprayed layer **2b** is stress concentration point. Since the breaking portion is determined as the starting point, it is possible to easily and firmly separate the layer **2a** for preventing noise electric wave. Furthermore, the adhesion of the layer **2a** for preventing noise electric wave to the electrode substrate **20** is improved by the substrate thermal sprayed layer **2b**. Therefore, it is possible to control the coming-off of the layer at the time of separating the layer **2a** for preventing noise electric wave.

## Embodiment 31

In the Embodiment 31, a rotor electrode **2** as the electrode for preventing noise electric wave is manufactured by the

## 26

fifth method according to claim 11. The materials for the electrode substrate **20** and the layer **2a** for preventing noise electric wave are the same as those of the Embodiment 26, and the layer **2a** for preventing noise electric wave has the porosity of 5% and the thickness of 400 microns.

As shown in the plan view of FIG. 25, an electrode substrate **20** having a key hole **23** with a key engaging portion **23a** is prepared. As shown in FIG. 26, a number of the electrode substrates **20** having the same thickness (1.6 mm) each other are laminated, and set in a swing apparatus which mainly comprises a fixed tool **4**, a swing tool **5**, a motor **6** and a cam shaft **7** as follows.

As shown in FIG. 27, the swing tool **5** is brought into contact with a cam portion **71** of the cam shaft **7** which is connected with the motor **6**, and it is swingable in the right and left directions (namely, in the direction vertical to the paper in FIG. 26; or in the up and down directions in FIG. 27) by the rotation of the cam shaft **7**. As shown in FIG. 28, the swing tool **5** has a bar portion **51** and a number of key portions **52**. The bar portion **51** is inserted through the key hole **23** of each laminated electrode substrate **20**, and the key portion **52** is engaged with the key engaging portion **23a** of the key hole **23** of every other laminated electrode substrate **20**. As shown in FIG. 29, concerning each electrode substrate **20** in which the key portion **52** is not engaged with the key engaging portion **23a** of the key hole **23**, the right and left side surfaces is restricted their movement in the right and left directions by a regulated wall surface **41** of the fixed tool **4**. Furthermore, concerning the laminated electrode substrates **20**, the upper surface of the electrode substrate **20** at the top and the lower surface of the electrode substrate **20** at the bottom are respectively covered by an upper wall surface **42** and a lower wall surface of the fixed tool **4**.

The cam shaft **7** is rotated by driving the motor **6**, and the swing tool **5** is swung. Then,  $\text{Al}_2\text{O}_3$ -60 wt % CuO material is thermal sprayed by plasma method in the direction which is perpendicular to the edge surface **24** of each electrode **20** while swinging only the electrode substrate **20** in which the key portion **52** is engaged with the key engaging portion **23a** of the key hole **23**.

The thermal spraying by plasma method is performed under the same condition as that of the Embodiment 26. The swing is performed under the condition that the swing frequency is 5 Hz, and the swing amplitude is 700 microns. The formation speed of the thermal sprayed layer is 100 microns per second, the thickness of the thermal sprayed layer which is formed during 1 cycle of swing is 20 microns. The average particle diameter of the thermal spraying material powder is 22 microns. After the thermal spraying material is thermal sprayed, it becomes flat and the average particle diameter is 70 microns. Therefore, the value of **s** (the swing amplitude) to **d** (the particle diameter after thermal spraying) is 10.

After that, the swing apparatus is removed from each electrode substrate **20**, and the rotor electrode **2** according to the Embodiment 31 is completed.  
(Relationship between the swing speed and the fraction defective of the thermal sprayed layer)

The relationship between the swing speed and the fraction defective of the thermal sprayed layer is examined under the above condition. The fraction defective is defined as the coming-off of the thermal sprayed layer or the crack in the layer due to swing. In order to examine the swing speed, it is necessary to consider the relationship with the formation speed of the thermal sprayed layer. Thus, the thickness of the thermal sprayed layer which is formed during 1 cycle of

swing is used to judge whether the condition of the swing speed is good or not. The result is shown in FIG. 30.

As shown in FIG. 30, when the thickness of the thermal sprayed layer which is formed during 1 cycle of swing is not more than 100 microns, it is possible to satisfactorily form the thermal sprayed layer with no fraction defective. (Relationship between the swing amplitude and the fraction defective of the thermal sprayed layer)

The relationship between the swing amplitude and the fraction defective of the thermal sprayed layer is examined under the above condition. In order to examine the swing amplitude, it is necessary to consider the relationship with the particle diameter of the thermal spraying material powder after thermal spraying. Thus, the value of s (the swing amplitude) to d (the particle diameter of the thermal spraying material after thermal spraying) is used to judge whether the condition of the swing amplitude is good or not. The result is shown in FIG. 31.

As shown in FIG. 31, when the value of s (the swing amplitude) to d (the particle diameter of the thermal spraying material after thermal spraying) is not less than 1, it is possible to satisfactorily form the thermal sprayed layer with no fraction defective.

#### Embodiment 32

In the Embodiment 32, a rotor electrode 2 as the electrode for preventing noise electric wave is manufactured by the sixth method according to claim 12. The materials for the electrode substrate 20 and the layer 2a for preventing noise electric wave are the same as those of the Embodiment 26, and the layer 2a for preventing noise electric wave has the porosity of 5% and the thickness of 400 microns.

A long-shaped electrode raw material having the same cross-sectional shape as that of the electrode substrate 20 is prepared. Then,  $\text{Al}_2\text{O}_3$ -60 wt % CuO material is thermal sprayed by plasma method to one surface of the electrode raw material in the perpendicular direction. The thermal spraying by plasma method is performed under the same condition as that of the Embodiment 26. After that, the thermal sprayed electrode raw material is cut in the direction perpendicular to the thermal sprayed surface by grinder for cutter to be the electrode substrate 20 having a certain thickness. Thus, the rotor electrode 2 according to the Embodiment 32 is completed.

In the method according to Embodiment 32, it is possible to prevent the formation of the porous thermal sprayed layer at least on the cut surface of the separated electrode substrate 20. Furthermore, it is possible to manufacture many electrodes productively. Moreover, the layer 2a for preventing noise electric wave is separated by machining at the time of cutting. Therefore, it is possible to control the coming-off of the layer 2a or slippage at the cut surface.

#### Embodiment 33

In the Embodiment 33, a rotor electrode 2 as the electrode for preventing noise electric wave is manufactured by the seventh method according to claim 13. The materials for the electrode substrate 20 and the layer 2a for preventing noise electric wave are the same as those of the Embodiment 26, and the layer 2a for preventing noise electric wave has the porosity of 5% and the thickness of 400 microns.

A number of the electrode substrates 20 which has the same shape as that of the Embodiment 26 are laminated in such a manner that the edge surface 24 is uniform surface, and the laminated electrode substrates 20 are set in a tool (not shown). The tool maintains the base edge side of each

laminated electrode substrate 20. The right and left side surfaces of each laminated electrode substrate 20, the upper surface of the electrode substrate 20 at the top and the lower surface of the electrode substrate 20 at the bottom are exposed at the tip side of each electrode substrate 20, namely, at the edge surface 24 on which thermal spraying is performed. Then,  $\text{Al}_2\text{O}_3$ -60 wt % CuO material is thermal sprayed by plasma method in the direction which is perpendicular to the edge surface 24 of each electrode 20. The thermal spraying by plasma method is performed under the same condition as that of the Embodiment 26. After that, the tool is removed and each electrode substrate is disassembled. The thermal sprayed layer formed on the surface of each electrode substrate 20 which is horizontal to the thermal spraying direction (the upper and lower surfaces and the right and left side surfaces of the stepped portion 20a) is fused and densified by laser irradiation. Thus, the rotor electrode 2 according to the Embodiment 33 is completed. The laser irradiation is performed under the condition that the laser output is 100 W, the laser pulse is 10 msec/pulse and 20 pulse/second, and the irradiation traverse speed is 1 cm/second. The porosity of the thermal sprayed layer before laser irradiation is about 50%, and the porosity of the thermal sprayed layer after laser irradiation is about 10%.

In the method according to Embodiment 33, the porous thermal sprayed layer formed on the surface of the electrode substrate 20 which is horizontal to the thermal spraying direction is densified by laser irradiation, and the porous portion of the thermal sprayed layer is firmly omitted. Therefore, it is possible to provide the electrode for preventing noise electric wave which can firmly prevent the generation of the micro discharge at the porous portion of the thermal sprayed layer. (Relationship between the porosity of the thermal sprayed layer formed on the surface of the electrode substrate which is horizontal to the thermal spraying direction and the effect for decreasing radio noise)

In the method according to the Embodiment 33, the laser output and the time for irradiation are changed, and the porosity of the thermal sprayed layer formed on the surface of the electrode substrate which is horizontal to the thermal spraying direction is variously changed, thereby manufacturing each rotor electrode. Concerning these rotor electrodes and the above completed rotor electrode 2, PNL operating time and radiation electric field intensity were measured. The result is shown in FIG. 32.

As shown in FIG. 32, the PNL operating time becomes short as the porosity of the above thermal sprayed layer is decreased. When the porosity is not more than 20%, the decreasing rate becomes almost constant. The radiation electric field intensity maintains a certain value without receiving the influence of the porosity of the thermal sprayed layer. As a result, when the porosity of the thermal sprayed layer is set to be not more than 20%, the PNL operating time is drastically decreased. Therefore, it is possible to decrease the radio noise without decreasing the effect for preventing noise electric wave.

FIG. 33 shows the result of examining PNL operating time and the induced discharge wave form before the porous thermal sprayed layer is fused. FIG. 34 shows the result of examining PNL operating time and the induced discharge wave form after the porous thermal sprayed layer is fused. As shown in FIGS. 33 and 34, it is possible to drastically decrease the PNL operating time and the radio noise.

In the Embodiment 33, not only the laser irradiation but also the electron beam is used as the means for fusing the thermal sprayed layer which is formed on the surface of the electrode substrate which is horizontal to the thermal spraying direction.

## Sixth Preferred Embodiment

## Embodiment 34

In the Embodiment 34, an electrode for preventing noise electric wave according to claim 14 is used as a rotor electrode 2.

As shown in the cross-sectional view of FIG. 35, the rotor electrode 2 according to the Embodiment 34 comprises an electrode substrate 20 made of brass having the thickness of 1.6 mm, a high-fusing conductive material layer 25 which is coated by thermal spraying on the surface of the electrode substrate 20 faced to a side electrode 3, a first resisting material layer 26 which is coated by thermal spraying on the surface of the high-fusing conductive material layer 25, and a second resisting material layer 27 which is coated by thermal spraying on the surface of the first resisting material layer 26.

The high-fusing conductive material layer 25 is made of Mo having the resistivity of  $5.7 \times 10^{-6}$  ohm centimeters and the fusing point of 2622° C. The thickness of the high-fusing conductive material layer 25 is 100 microns.

The first resisting material layer 26 is made of  $\text{Al}_2\text{O}_3$ -13%  $\text{TiO}_2$ . The thickness of the first resisting material layer 26 is 400 microns.

The second resisting material layer 27 is made of  $\text{Al}_2\text{O}_3$ . The thickness of the second resisting material layer is 50 microns.

The high-fusing conductive material layer 25, the first resisting material layer 26 and the second resisting material layer 27 are formed by Plasma thermal spraying method. After thermal spraying, the upper and lower surfaces of the electrode substrate 20 are ground, and the porous thermal sprayed layer formed on the upper and lower surfaces of the electrode substrate 20 is removed.

## Embodiment 9

In order to confirm the effect of the formation of the high-fusing conductive material layer 25, a rotor electrode according to the Embodiment 9 is prepared. The rotor electrode comprises an electrode substrate which is made of brass; a first resisting material layer (first layer) which is made of  $\text{Al}_2\text{O}_3$ -13%  $\text{TiO}_2$ , and which is coated by thermal spraying on the surface of the electrode substrate, and which has the thickness of 400 microns; and a second resisting material layer (second layer) which is made of  $\text{Al}_2\text{O}_3$ , and which is coated by thermal spraying on the surface of the electrode substrate, and which has the thickness of 50 microns.

## Embodiment 35

In order to confirm the effect of the formation of the high-fusing conductive material layer 25, a rotor electrode is prepared. The rotor electrode is the same as that of the Embodiment 9 except that the electrode substrate is made of Mo.

## (Evaluation of durability)

Concerning each rotor electrode according to the Embodiment 34, 9 and 35, an endurance test is performed while each rotor electrode is used for 0 to 800 hours, and noise electric wave having 180 mHz was measured by an actual vehicle. The result is shown in FIG. 36.

As shown in FIG. 36, concerning the rotor electrode according to the Embodiment 34 in which the high-fusing conductive material layer 25 is disposed between the first resisting material layer 26 and the electrode substrate 20, it

is possible to maintain the initial performance for preventing noise electric wave after the rotor electrode has been used for 800 hours. On the contrary, concerning each rotor electrode according to the Embodiments 9 and 35 with no high-fusing conductive material layer 25, the performance for preventing noise electric wave is deteriorated after each rotor electrode has been used for 800 hours. The rotor electrode of the Embodiment 35 in which the electrode substrate is made of Mo having higher fusing point than that of brass has lower decreasing speed in performance for preventing noise electric wave than that of the Embodiment 9 in which the electrode substrate is made of brass. However, both of these rotor electrodes show the same deteriorated performance at last.

15 (Relationship between the thickness of the high-fusing conductive material layer and the level of noise electric wave)

Concerning the rotor electrode according to the Embodiment 34, the relationship between the thickness of the high-fusing conductive material layer 25 and the level of noise electric wave was examined. The result is shown in FIG. 37. The endurance test which is the same as above was performed, and noise electric wave having 180 mHz was measured.

As seen from FIG. 37, there is an appropriate thickness of the high-fusing conductive material layer 25 for improving the durability of the performance for preventing noise electric wave. When the thickness of the high-fusing conductive material layer 25 is less than 30 microns, the effect for improving the durability due to the high-fusing conductive material layer 25 cannot be satisfactorily achieved. Therefore, it is necessary that the thickness of the high-fusing conductive material layer 25 is not less than 30 microns, preferably, not less than 70 microns. When the high-fusing conductive material layer 25 becomes too thick, it is preferable that the thickness is not more than 200 microns since coming-off of the layer is generated.

## Seventh Preferred Embodiment

## Embodiment 36

40 In the Embodiment 36, an electrode for preventing noise electric wave according to claim 17 is used as a rotor electrode 2.

As shown in the cross-sectional view of FIG. 38, the rotor electrode 2 according to the Embodiment 36 comprises an electrode substrate 20 made of brass, a first resisting material layer 26 which is coated by thermal spraying on the surface of the electrode substrate 20 faced to a side electrode, and a second resisting material layer 27 which is coated by thermal spraying on the surface of the first resisting material layer 26.

45 The electrode substrate 20 has a covering portion 28 which is covered on the upper and lower surfaces of the first resisting material layer 26, and which is located at the connecting portion between the electrode substrate and the first resisting material layer 26. The thickness a of the covering portion is 0.2 mm, and the length b of the covering portion is 0.5 mm.

50 The first resisting material layer 26 is made of  $\text{Al}_2\text{O}_3$ -13%  $\text{TiO}_2$ . The thickness of the first resisting material layer 26 from the edge surface of the covering portion 28 is 400 microns.

55 The second resisting material layer 27 is made of  $\text{Al}_2\text{O}_3$ . The thickness of the second resisting material layer 27 is 50 microns.

60 The first resisting material layer 26 and the second resisting material layer 27 are formed by Plasma thermal

## 31

spraying method on the electrode substrate **20** on which the covering portion **28** is previously formed. After thermal spraying, the upper and lower surfaces of the electrode substrate **20** are ground, and the porous thermal sprayed layer formed on the upper and lower surfaces of the electrode substrate **20** is removed. Therefore, the thickness of the electrode substrate **20** is 1.0 mm.

## Embodiment 9

In order to confirm the effect of the formation of the covering portion **28**, a rotor electrode according to the Embodiment 9 is prepared. The rotor electrode comprises an electrode substrate with no covering portion **28** which is made of brass; a first resisting material layer (first layer) which is made of  $Al_2O_3$ -13%  $TiO_2$ , and which is coated by thermal spraying on the surface of the electrode substrate, and which has the thickness of 400 microns; and a second resisting material layer (second layer) which is made of  $Al_2O_3$ , and which is coated by thermal spraying on the surface of the electrode substrate, and which has the thickness of 50 microns.

## (Evaluation of durability)

Concerning each rotor electrode according to the Embodiments 9 and 36, an endurance test is performed while each rotor electrode is used for 0 to 800 hours, and noise electric wave having 180 mHz is measured by an actual vehicle. The result is shown in FIG. 39.

As shown in FIG. 39, concerning the rotor electrode according to the Embodiment 36 in which the covering portion **28** is formed between the first resisting material layer **26** and the electrode substrate **20**, the performance for preventing noise electric wave becomes deteriorated to some extent until 100 hours. After that, it is possible to maintain almost constant performance, and this is acceptable as compared with the law regulating level. On the contrary, concerning the rotor electrode according to the Embodiment 9 with no covering portion **28**, the performance for preventing noise electric wave becomes deteriorated to show the higher level than the law regulating level until 100 hours, and is further deteriorated until 400 hours.

(Relationship between the thickness of the covering portion and the level of noise electric wave)

Concerning the rotor electrode according to the Embodiment 36, the relationship between the thickness *a* of the covering portion **28** and the level of noise electric wave is examined. The result is shown in FIG. 40. The endurance test which is the same as above is performed, and noise electric wave having 180 mHz is measured after the rotor electrode has been used for 400 hours.

As seen from FIG. 40, there is an appropriate thickness *a* of the covering portion **28** for improving the durability of the performance for preventing noise electric wave. When the thickness *a* of the covering portion **28** is more than 0.34 mm, the performance for preventing noise electric wave shows the higher level than the law regulating level. Therefore, it is preferable that the thickness *a* of the covering portion **28** is not more than 0.34 mm, more preferably, not more than 0.25 mm. When the thickness *a* of the covering portion **28** becomes too thin, it is preferable that the thickness is not less than 0.1 mm since the speed for progressing fused loss becomes high.

It is necessary that the length *b* of the covering portion **28** is not less than 0.1 mm per 50000 km of the travel distance of an automobile. Therefore, it is preferable that the length *b* of the covering portion **28** is not less than 0.1 mm, more preferably, not less than 0.6 mm.

## Eighth Preferred Embodiment

## Embodiment 37

In the Embodiment 37, an electrode for preventing noise electric wave according to claim 5 is used as a rotor electrode **2**.

## 32

The rotor electrode **2** according to the Embodiment 37 comprises a substrate **20** made of brass, a substrate layer **21** formed on the surface of the substrate **20**, a first layer **22** formed and coated on the surface of the substrate layer **21** and a second layer **23** formed on the surface of the first layer **22**.

The substrate layer **21** is formed in such a manner that the first layer **22** is firmly adhered to the substrate **20** by thermal spraying. The substrate layer **21** is made of Ni-5% Al alloy and has the thickness of 50 microns. The substrate layer **21** is formed by plasma spraying method.

The first layer **22** is made of  $Al_2TiO_5$ -70 wt %  $Al_2O_3$  and has the thickness of 400 microns. The first layer **22** is formed by plasma spraying method. The direct current resistance value  $R_1$  of the first layer **22** is in the range of  $10^9$  ohm.

The second layer **23** is formed by performing heat-oxidation treatment due to plasma flame on the surface of the first layer **22**. The second layer **23** has the thickness of about 10 microns. The direct current resistance value  $R_2$  of the second layer **23** is in the range of  $10^{10}$  ohm.  $Al_2TiO_5$  is changed from insulating material to resisting material since oxygen defect is generated by plasma spraying. After that,  $Al_2TiO_5$  is changed from resisting material to insulating material again because oxygen is supplied by oxidation treatment.

In the rotor electrode **2** according to the Embodiment 37, the first layer **22** is coated on the surface of the substrate **20**, and the second layer **23** is formed on the surface of the first layer **22** by performing oxidation treatment on the surface of the first layer **22**. After that, the upper and lower surfaces of the electrode are polished, and a porous thermal sprayed layer formed on the upper and lower surfaces is removed. Thus, the rotor electrode **2** is completed.

The following is the reason why the porous thermal sprayed layer formed on the upper and lower surfaces is removed. When the porous thermal sprayed layer exists around the place where discharge is generated (the upper and lower surfaces of the electrode), discharge electron is likely to remain in the space between thermal sprayed particles. The time for discharge becomes long so that noise is likely to occur in the radio which is loaded on automobiles.

## Embodiment 38

In the Embodiment 38, a first layer **22** is coated and formed on the surface of a substrate layer **21** of a substrate **20** by plasma spraying method in the same manner as that of the Embodiment 37. Then, a second layer **23** is coated and formed on the surface of the first layer **22** by plasma spraying method. The second layer **23** is made of  $Al_2O_3$  and has the thickness of about 10 microns. After that, the upper and lower surfaces of the electrode are polished, and a porous thermal sprayed layer is removed in the same manner as that of the Embodiment 37. Thus, a rotor electrode **2** according to the Embodiment 38 is completed.

## Embodiment 39

In the Embodiment 39, a rotor electrode **2** is manufactured by the same method according to the Embodiment 38 except that the first layer **22** is made of  $TiO_2$ -70 wt %  $Al_2O_3$  and has the thickness of 400 microns.

## Embodiment 40

In the Embodiment 40, a rotor electrode **2** is manufactured by the same method according to the Embodiment 38 except that the first layer **22** is made of  $TiO_2$ -15 wt %  $Al_2TiO_5$ -70 wt %  $Al_2O_3$  and has the thickness of 400 microns.

## 33

## Comparative Example 1

A rotor electrode **2** according to Comparative Example 1 comprises only a substrate which is made of brass.

## Comparative Example 6

In Comparative Example 6, a rotor electrode **2** is manufactured by the same method according to the Embodiment 37 except that only an insulation layer is formed on the surface of the substrate layer **21**. The insulating layer is made of  $\text{Al}_2\text{O}_3$  (99.7%) and has the thickness of 400 microns.

## Comparative Example 8

In Comparative Example 8, a rotor electrode **2** is manufactured by the same method according to the Embodiment 37 except that the first layer **22** is made of  $\text{CuO}$ -40 wt %  $\text{Al}_2\text{O}_3$  and has the thickness of 400 microns, and the second layer **23** is not formed.

## Comparative Example 9

In Comparative Example 9, a rotor electrode **2** is manufactured by the same method according to the Embodiment 39 except that the second layer **23** is not formed.

## Comparative Example 10

In Comparative Example 10, a rotor electrode **2** is manufactured by the same method according to the Embodiment 40 except that the second layer **23** is not formed.

(Evaluation)

Concerning each electrode, the decreasing amount of the level of noise electric wave (decreasing amount of noise) having 180 MHz was measured at the initial stage and at 500 hours later. The result is shown in FIG. 41. This measurement was performed under the condition that the temperature was ordinary temperature, and that the engine speed was 1500 rpm.

In the above measurement, each electrode according to the Embodiments 37 and 38 show the excellent effect for preventing noise electric wave not only at the initial stage but also at 500 hours later. Concerning each electrode according to the Embodiments 37 and 38, the condition for generating discharge was enlarging photographed by high-speed video (0.001 sec/frame). The result is shown in FIG. 42.

As shown in FIG. 42, discharge is generated from the boundary portion between the substrate **20** and the first layer **22**. The discharge passage is extended toward the opposite electrode (cathode) **3** along the upper and lower surfaces and the tip surface of the electrode, and creeping discharge can be observed. Thus, when electron is moved on the creeping surface of the first layer **22** and the second layer **23** having high electric resistance, discharge energy is damped, thereby decreasing the generation of electric/magnetic field which causes noise. Furthermore, in each electrode according to the Embodiments 37 and 38, metal oxide in the first layer **22** exists as composite oxide such as  $\text{Al}_2\text{TiO}_5$ , and it contributes to the effect for preventing noise electric wave. Namely, when the component elements of  $\text{Al}_2\text{TiO}_5$  such as Ti and O exist as  $\text{TiO}_2$  having low electric resistance, the second layer **23** is broken, thereby generating discharge. At that time, the second layer **23** is fused and damaged. After that, discharge is generated from the tip surface of the second layer **23**, and the effect for preventing noise electric wave is deteriorated. On the contrary, when metal oxide in the first layer **22** exists as composite oxide such as  $\text{Al}_2\text{TiO}_5$ , the above discharge passage and the effect for preventing noise electric wave can

## 34

be obtained since  $\text{Al}_2\text{TiO}_5$  shows higher electric resistance than that of  $\text{TiO}_2$ . Furthermore, in each electrode according to the Embodiments 37 and 38, the second layer **23** exists as an insulation layer. As a result, when electron of creeping discharge is moved toward the opposite electrode (cathode) **3**, as shown in FIG. 43, the outflow of electron charged in oxide resistor **22** in the first layer **22** can be prevented by the second layer **23**. Therefore, it is possible to prevent increasing in discharge current value due to outflow of electron, and to prevent increasing in noise electric wave.

A thermal sprayed layer is formed on the tip surface of the substrate **20** by plasma spraying method. The substrate **20** is made of brass, and the thermal sprayed layer is made of  $\text{Al}_2\text{TiO}_5$  and has the thickness of 0.4 mm. Then, the direct current resistance value of  $\text{Al}_2\text{TiO}_5$  was measured by an ammeter when the voltage of 100V was acted on a boundary portion between the upper surface of the substrate **20** and the tip surface of the thermal sprayed layer. As a result, the direct current resistance value was in the range of  $1 \times 10^6$  to  $1 \times 10^7$  ohm. Similarly, the direct current resistance value of  $\text{TiO}_2$  was 10 ohm, and  $\text{Al}_2\text{O}_3$  was  $1 \times 10^{12}$  ohm. (Relationship between the thickness of the second layer **23** and the effect for preventing noise electric wave)

In the above Embodiment 38, while the total thickness of the first layer **22** and the second layer **23** is 0.4 mm, the thickness of the second layer **23** is variously changed. Then, the decreasing amount of the level of noise electric wave (decreasing amount of noise) having 180 MHz was measured at the initial stage and at 500 hours later. The result is shown in FIG. 44. This measurement was performed under the condition that the temperature was ordinary temperature, and that the engine speed was 1500 rpm.

In the above measurement, when the thickness of the second layer **23** is more than 25 microns, there is no problem on the initial noise characteristics. However, the level of noise is radically increased at 500 hours later. The reason of this is as follows. When the thickness of the second layer **23** is more than 25 microns, impedance of whole electrode becomes high. So, heating energy becomes high at the place for generating discharge, and the local place is fused and damaged. Therefore, it is preferable that the thickness of the second layer **23** is not more than 25 microns. Since the second layer **23** is used for preventing the outflow of electron from oxide resistor of the first layer **22**, it is no problem that the second layer **23** is thin.

In each electrode for preventing noise electric wave according to claims 1 to 19, it is possible to prevent noise electric wave for a long time. As a result, other step for preventing noise electric wave such as a bonding wire is not required, so it is possible to decrease the cost and the manhour. Furthermore, since each electrode has the same noise level as that of a ceramic rotor electrode which is expensive, it is possible to use each electrode as a substitution for the ceramic rotor electrode. Therefore, it is possible to lower the cost remarkably.

The electrodes for preventing noise electric wave according to claims 1 to 4 comprises the first layer comprising oxide resistor and the second layer comprising oxide resistor, and the resistivity of the second layer located at outside is larger than that of the first layer. Therefore, it is possible to effectively prevent the generation of noise electric wave as compared with the conventional electrode which has a single layer comprising high electrical resistance substance.

The electrode for preventing noise electric wave according to claim 3 shows further effect for preventing noise electric wave due to the effect of creeping discharge and the

effect for preventing outflow of electron caused by the second layer which is functioned as the insulating layer.

The electrode for preventing noise electric wave according to claim 4 has the same construction as that of the electrode according to claim 3 except that the second layer comprises both the oxide resistor and the oxide dielectric substance. As a result, the resistivity of the second layer is decreased, and the performance of the barrier at the time of discharge is decreased. Therefore, it is possible to prevent the generation of pin hole, and to improve the durability.

In each electrode for preventing noise electric wave according to claims 6 to 12, the generation of relatively large induction discharge current which is caused by the micro discharge at the porous portion of the thermal sprayed layer can be controlled. As a result, it is possible to prevent the radio noise which is caused by the induction discharge current.

In the first and seventh methods for producing the electrode according to claims 7 and 13, it is possible to firmly form the layer for preventing noise electric wave which comprises only a thermal sprayed layer having the porosity of not more than 20%.

In the second to fifth methods for producing the electrode according to claims 8 to 11, since thermal spraying is performed at each edge surface of a number of laminated electrode substrates, it is possible to prevent the formation of the porous thermal sprayed layer at least on the overlapping surface made by two neighboring electrode substrates. At the same time, it is possible to manufacture many electrodes productively, and to lower the cost.

In the third method for producing the electrode according to claim 9, each layer for preventing noise electric wave formed on each electrode substrate is previously separated by each spacer. Therefore, it is possible to control coming-off of the layer at the time of separating the layer for preventing noise electric wave, and to improve the quality.

In the fourth method for producing the electrode according to claim 10, when the layer for preventing noise electric wave is separated along a dividing line of each electrode substrate, a breaking portion of a substrate thermal sprayed layer is used as a starting point. Therefore, it is possible to easily and firmly separate the layer for preventing noise electric wave, and to improve the quality.

In the fifth method for producing the electrode according to claim 11, since thermal spraying is performed, and at the same time, the electrode substrate is swung, the layer for preventing noise electric wave formed on each electrode substrate is not adhered to each other. As a result, it is possible to omit the process for separating the layer for preventing noise electric wave, and to prevent coming-off of the layer in the process for separating the layer. Furthermore, it is possible to improve the quality.

In the sixth method for producing the electrode according to claim 12, the layer for preventing noise electric wave is formed on one surface of long-shaped electrode substrate, and then the long-shaped electrode substrate is cut into many pieces. Therefore, it is possible to prevent the formation of the porous thermal sprayed layer at least on the cut surface of each electrode substrate, and to manufacture many electrodes productively, and to lower the cost. Furthermore, it is possible to prevent coming-off or slippage of the layer since the layer for preventing noise electric wave is separated by machining at the time of cutting.

In the electrode for preventing noise electric wave according to claim 14, since the high-fusing conductive material layer exists between the substrate and the resisting material layer, the portion for the discharge generation is moved from

the substrate to the high-fusing conductive material layer. Therefore, it is possible to prevent the generation of fused loss which causes increase in noise electric wave.

In the electrode for preventing noise electric wave according to claim 15, the substrate comprises copper or copper alloy having high heat conductivity. As a result, it is possible to control fused loss at the high-fusing conductive material layer due to outgoing radiation from the substrate, and to improve the durability.

In the electrode for preventing noise electric wave according to claim 17, the substrate has the covering portion which is covered on the resisting material layer. Therefore, the damage of fused loss which causes the increase in noise electric wave is checked by the thickness of the covering portion, and it is possible to improve the durability.

In each electrode for preventing noise electric wave according to claims 18 and 19, since the above covering portion has a certain dimension, it is possible to further improve the durability.

Having now fully described the present invention, it will be apparent to one of ordinary skill in the art that many changes and modifications can be made thereto without departing from the spirit or scope of the present invention as set forth herein including the appended claims.

What is claimed is:

1. A low electric noise electrode system, comprising:  
a first electrode and a metal second electrode separated  
from the first electrode by an air gap;  
said first electrode comprising,

a metal electrode substrate,  
a first layer comprising a material selected from the group  
consisting of a metal oxide, an oxide resistor, and a  
mixture of an oxide dielectric substance and an oxide  
resistor, said first layer formed on a surface of said  
substrate; and

a second layer comprising a material of which said first  
layer is formed but having a larger resistivity than that  
of said first layer, said second layer being formed on  
the surface of said first layer covering said first layer and  
having an exposed surface placed opposite said second  
electrode with said air gap between the exposed surface  
of the second layer and the second electrode so as to  
conduct a discharge between said exposed surface and  
said second electrode upon application of a sufficiently  
high voltage across said exposed surface and said  
second electrode.

2. A low electric noise rotor electrode system for an  
automotive distributor rotor, comprising:

a first electrode and a metal second electrode separated  
from the first electrode by an air gap;  
said first electrode comprising,

a metal electrode substrate,  
a first layer comprising a material selected from the group  
consisting of a metal oxide, an oxide resistor, and a  
mixture of an oxide dielectric substance and an oxide  
resistor, said first layer formed on the surface of said  
substrate, and

a second layer comprising a material of which said first  
layer is formed but having a larger resistivity than that  
of said first layer, said second layer being formed on  
the surface of said first layer covering said first layer and  
having an exposed surface placed opposite said second  
electrode with the air gap between the exposed surface  
of the second layer and the second electrode so as to  
conduct a discharge between said exposed surface and

said second electrode upon application of a sufficiently high voltage across said exposed surface and said second electrode.

3. The low electric noise electrode system of claim 1, wherein the first layer has a surface facing said second electrode and the entire surface of said first layer facing said second electrode is covered by the second layer of the first electrode. 5

4. The low electric noise rotor electrode system of claim 2, wherein the first layer has a surface facing said second electrode and the entire surface of said first layer facing said second electrode is covered by the second layer of the first electrode. 10

5. An electrode for preventing noise electric wave according to the present invention comprising:

a substrate; 15  
a first layer comprising oxide dielectric substance and oxide resistor, and being formed on the surface of said substrate faced to an opposite electrode; and  
a second layer comprising oxide dielectric substance, and being formed on the surface of said first layer faced to said opposite electrode, and having larger resistivity than that of said first layer. 20

6. An electrode for preventing noise electric wave according to the present invention comprising:

a substrate; 25  
a high-fusing conductive material layer which is formed on the surface of said substrate faced to an opposite electrode, and which has the resistivity of not more than  $10^4$  ohm centimeters, the fusing point of not less than 2000° C., and the thickness of not less than 30 microns; and  
not less than one resisting material layer which is coated on the surface of said high-fusing conductive material layer faced to said opposite layer. 30

7. An electrode for preventing noise electric wave according to claim 6, wherein said substrate comprises copper or copper alloy. 35

8. An electrode for preventing noise electric wave according to claim 6 or 7, wherein said high-fusing conductive material layer comprises not less than one kind of materials consisting of Mo, Ta, W,  $\text{Cr}_2\text{O}_3$  and  $\text{CeO}_2$ . 40

9. An electrode for preventing noise electric wave according to the present invention comprising:

a substrate; and 45  
a resisting material layer which is coated on the surface of said substrate faced to an opposite electrode; wherein said substrate has a covering portion which is covered on the outer periphery of said resisting material layer, and which is located at the connecting portion between said substrate and said resisting material layer. 50

10. An electrode for preventing noise electric wave according to claim 9, wherein said coating portion of said substrate is not more than 0.34 mm. 55

11. An electrode for preventing noise electric wave according to claim 9 or 10, wherein the length of said coating portion of said substrate is not less than 0.1 mm. 55

12. An electrode for preventing noise electric wave according to the present invention comprising:

a substrate; and 60  
a layer for preventing noise electric wave comprising a thermal sprayed layer, and being coated on the surface of said substrate faced to an opposite electrode, and having the porosity of not more than 20%. 65

13. A method for producing an electrode for preventing noise electric wave according to the present invention comprising:

a process for forming a first layer which comprises metal oxide on the surface of a substrate faced to an opposite electrode; and

a process for forming a second layer which comprises metal oxide and has larger resistivity than that of said first layer on the surface of said first layer faced to said opposite electrode by performing oxidation treatment on the surface of said first layer.

14. A method for producing an electrode for preventing noise electric wave according to the present invention comprising:

a process for forming a layer for preventing noise electric wave comprising a thermal sprayed layer which is formed on one surface of a substrate, and in which thermal spraying is performed in the direction approximately perpendicular to the surface, and which has the porosity of not more than 20%; and

a process for removing said thermal sprayed layer in which thermal spraying is performed on the other surface of said substrate, and which has the porosity of more than 20%.

15. A method for producing an electrode for preventing noise electric wave according to the present invention comprising:

a process for laminating a number of substrates; 25  
a process for forming a layer for preventing noise electric wave comprising a thermal sprayed layer which is formed on each edge surface of each substrate, and in which thermal spraying is performed in the direction approximately perpendicular to each edge surface, and which has the porosity of not more than 20%; and

a process for separating said layer for preventing noise electric wave along a dividing line of each electrode substrate.

16. A method for producing an electrode for preventing noise electric wave according to the present invention comprising:

a process for laminating a number of substrates having a spacer therebetween in which edge portion of each spacer is projected from the edge surface of each substrate by the predetermined length;

a process for forming a layer for preventing noise electric wave comprising a thermal sprayed layer which is formed on each edge surface of each substrate, and in which thermal spraying is performed in the direction approximately perpendicular to each edge surface in such a manner that the thickness of said thermal sprayed layer is thinner than said predetermined length, and which has the porosity of not more than 20%; and

a process for tearing said layer for preventing noise electric wave off from each spacer.

17. A method for producing an electrode for preventing noise electric wave according to the present invention comprising:

a process for laminating a number of substrates; 55  
a process for forming a substrate thermal sprayed layer which is formed on each edge surface of each substrate, and in which thermal spraying is performed in the direction approximately perpendicular to each edge surface;

a process for separating said substrate thermal sprayed layer along a dividing line of each substrate;

a process for re-laminating each substrate coated with said substrate thermal sprayed layer;

a process for forming a layer for preventing noise electric wave comprising a thermal sprayed layer which is

**39**

coated on said substrate thermal sprayed layer formed on each edge surface of each substrate, and in which thermal spraying is performed in the direction approximately perpendicular to each edge surface of re-laminating substrate, and which has the porosity of 5 not more than 20%; and

a process for separating said layer for preventing noise electric wave along a dividing line of each substrate.

**18.** A method for producing an electrode for preventing noise electric wave according to the present invention comprising: 10

a process for laminating a number of substrates; and

a process for forming a layer for preventing noise electric wave comprising a thermal sprayed layer which is formed on each edge surface of each substrate; and in which thermal spraying is performed in the direction approximately perpendicular to each edge surface, and at the same time, said substrate is swung in order to repeat relative displacement between two edge surfaces 15 of two neighboring substrates; and which has the porosity of not more than 20%. 20

**19.** A method for producing an electrode for preventing noise electric wave according to the present invention comprising:

**40**

a process for forming a layer for preventing noise electric wave comprising a thermal sprayed layer which is formed on one surface of long-shaped substrate, and in which thermal spraying is performed in the direction approximately perpendicular to said surface, and which has the porosity of not more than 20%; and

a process for cutting said long-shaped substrate into many pieces in the direction perpendicular to said surface.

**20.** A method for producing an electrode for preventing noise electric wave according to the present invention comprising:

a process for forming a layer for preventing noise electric wave comprising a thermal sprayed layer which is formed on one surface of said substrate, and in which thermal spraying is performed in the direction approximately perpendicular to said surface, and which has the porosity of not more than 20%; and

a process for fusing said thermal sprayed layer in which thermal spraying is performed on the other surface of said substrate, and which has the porosity of more than 20% by means of high density energy to be densified.

\* \* \* \* \*